

[54] **PROCESS OF TREATING FIBROUS ARTICLES WITH MICROCAPSULES CONTAINING HYDROPHOBIC TREATING AGENT**[75] Inventors: **Syunya Ida, Nara; Kenjiro Hosokawa, Osaka, both of Japan**[73] Assignee: **Kanegafuchi Boseki Kabushiki Kaisha, Tokyo, Japan**[22] Filed: **Sept. 26, 1972**[21] Appl. No.: **292,414****Related U.S. Application Data**

[63] Continuation of Ser. No. 65,244, Aug. 19, 1970, abandoned.

[30] **Foreign Application Priority Data**

Aug. 22, 1969 Japan..... 44-66574

Aug. 23, 1969 Japan..... 44-66786

Aug. 25, 1969 Japan..... 44-67429

Oct. 15, 1969 Japan..... 44-82727

[52] **U.S. Cl.**..... **117/33.3, 8/79, 8/115.5, 117/33.5 T, 117/136, 117/139.4, 117/140 R, 117/141, 117/143 R, 117/144, 117/161 KP, 117/161 ZB**[51] **Int. Cl.**..... **B44d 5/06**[58] **Field of Search**..... **117/100 A, 100 C, 139.5 A, 117/139.5 CQ, 139.4, 143 R, 136, 138.8 B, 137, 140 R, 141, 142, 144, 154, 161 ZB, 161**

KP, 35.5 T, 33.3; 252/316; 8/115.5

[56]

**References Cited****UNITED STATES PATENTS**

|           |         |                      |            |
|-----------|---------|----------------------|------------|
| 3,041,288 | 7/1962  | Anthony .....        | 117/36.2 X |
| 3,257,267 | 6/1966  | Hay.....             | 252/316 X  |
| 3,415,758 | 12/1968 | Powell et al. ....   | 252/316    |
| 3,632,296 | 1/1972  | Pandell et al. ....  | 8/115.5    |
| 3,660,321 | 5/1972  | Praetzel et al. .... | 252/8.1 X  |

*Primary Examiner*—William D. Martin*Assistant Examiner*—Theodore G. Davis*Attorney, Agent, or Firm*—Woodhams, Blanchard and Flynn

[57]

**ABSTRACT**

A fibrous article such as yarn, woven and knitted fabric and non-woven fabric is treated with hydrophobic treating agent by applying microcapsules composed of a core constituent consisting of a non-aqueous solvent solution of the hydrophobic treating agent and a wall constituent containing the core constituent and made up of a thin synthetic resin shell and having a low tenacity at break of at most 100 g/cm<sup>2</sup>, and then by breaking the applied microcapsules at a breaking force of at least 100 g/cm<sup>2</sup> so as to impregnate the fibrous article with the non-aqueous solvent solution which flows out from the broken microcapsules.

**18 Claims, No Drawings**

**PROCESS OF TREATING FIBROUS ARTICLES  
WITH MICROCAPSULES CONTAINING  
HYDROPHOBIC TREATING AGENT**

This is a continuation, of application Ser. No. 65,244, filed Aug. 19, 1970, now abandoned.

The present invention relates to a process of treating fibrous articles with microcapsules containing hydrophobic treating agent and, particularly, relates to a process of treating fibrous articles such as yarn, woven and knitted fabrics and non-woven fabric with microcapsules containing a nonaqueous solvent solution of hydrophobic treating agent.

Generally, it is already known that the microcapsules containing a hydrophobic liquid are prepared by the following methods.

1. Coacervation method in which electrolytic polymer such as gelatin and gum arabic is used as a protective colloid.

2. Interfacial polymerization method which is utilized for preparation of synthetic resin such as polyesters, polyurethanes, polyamides and polystyrene.

3. Phase separation method which is carried out in a three component system containing cellulose derivatives such as ethyl cellulose, solvent for polymer and non-solvent.

The microcapsules prepared through the conventional methods mentioned above are applied to several uses such as pressure sensitive paper which is the so-called no-carbon paper and ink for ball point pens. The conventional microcapsules prepared by the conventional process have sufficient tenacity, water proof property and stability only for the above-mentioned usual uses. When the conventional microcapsules are applied to treatment of the fibrous articles such as yarn, net, woven and knitted fabric and non-woven fabric, it is industrially very difficult to uniformly impregnate the fibrous article with the solution contained in the microcapsules because of the tenacity of the microcapsules is so great that breakage of the microcapsules is very difficult.

The conventional method for preparing the microcapsules had disadvantages such as the size of the resultant microcapsules is non-uniform and that when polyurethanes or epoxy resins are used for forming the shell of the microcapsule together with amine type hardening agent, the resultant microcapsules have a tendency to change color with lapse of time. In view of these disadvantages, it is unfavorable that the conventional microcapsules are applied to the field of treatment of fibrous articles.

On the other hand, in the field of treatment of fibrous articles, the new technique using a non-aqueous solvent is the so-called non-aqueous treatment process in which the treating agent is dissolved in the non-aqueous solvent. The non-aqueous treatment is effective for obtaining dyed or finished fibrous articles having excellent qualities at a low cost and to solve problems of waste water-discharging which have been recently brought into question.

However, the following disadvantages are found in the non-aqueous treatment process.

1. The solvent has frequently high toxicity to humans or a bad smell.

2. The solvent has frequently high corrosion property for the container.

3. Thus, the solvent container and the solvent solution of the treating agent and the treating apparatus

must be gas-tightly closed in order to protect workers from the toxicity or the odor.

When the fibrous article consists of two or more kinds of fibers, or when the fibrous article is subjected to two or more kinds of treatments, it is frequently required to mix two or more treating agents with each other in a treating bath. If the treating agents have no or a low miscibility with each other or if there is insufficient stability of the mixture, the treating agents should be separately applied to the fibrous articles.

An object of the present invention is to provide a process of treating fibrous articles with microcapsules having a low tenacity at break and containing a nonaqueous solvent solution of hydrophobic treating agent using an open treating apparatus.

Another object of the present invention is to provide a process of treating the fibrous article for two or more purposes by using the microcapsules containing the non-aqueous solvent solution of treating agent, which process can be performed easily and at low cost.

Further objects and features of the present invention will be illustrated by the detailed description set forth hereinbelow.

25 The term "microcapsule" as used herein refers to a specific capsule having a very small size and being composed of a core constituent consisting of a liquid and a wall constituent covering the liquid.

According to the present invention, the microcapsule 30 has a tenacity at break of at most 50 g/cm<sup>2</sup> and comprises a core constituent consisting of a solution of a hydrophobic agent for treating the fibrous articles in a non-aqueous solvent and a wall constituent covering the core constituent and being composed of a thin synthetic resin shell.

The microcapsule is prepared through the following process. A non-aqueous solvent solution containing a polymerizing compound such as prepolymer, polymerizable monomer and existing polymer and a desired 40 treating agent is dispersed in an aqueous solution containing dispersing agent or protective colloid and hardening agent for the polymerizing compound or in water. Generally, the dispersing is carried out by slowly 45 dropping the non-aqueous solvent solution into the aqueous solution or water while vigorously stirring. In this dispersion, the polymerizing compound is interfacially polymerized at the interfaces between the dispersed particles of the non-aqueous solvent solution 50 and the aqueous solution or water. The interfacially polymerized polymer forms the wall constituent of the microcapsules. The wall constituent contains the non-aqueous solvent solution of the treating agent forming a core constituent.

55 The treating agent usable for the present invention may be selected from compounds effective for treating the fibrous articles for the desired purpose. The treating agent may be adhered, absorbed or reacted with the fibrous article so as to improve or modify the chemical or physical property of the fibrous article. The treating agent may include, for example, elasticity improving agent, antipilling agent, flame proof agent, pleating agent, ultra-violet ray absorber, anti-static agent, soil proof agent, water repellent agent, crease proof agent, oil repellent agent, antishrinking agent, heat proof agent, softening agent, cross-linking agent, reactive monomer, coloring material such as dye and pigment.

The elasticity improving agent may be selected from poly-organosiloxane diols and the antipilling agent may be selected from urethane prepolymers.

The ultra-violet ray absorber may be selected from benzophenone type compounds, for example, 2,2'-4,4'-dimethoxy benzophenone, 2,2'-dihydroxy-4,4'-dimethoxy benzophenone, and 2-hydroxy-octoxy benzophenone. The softening agent may be dimethyl polysiloxane and dimethyl-polysiloxane diol, and the flame proof agent may be tris-(2-bromoethyl) phosphate, tris-(2-chloroethyl) phosphate, tris-(dichloropropyl) phosphate, tris-(2,3-dibromopropyl) phosphate, bis-(2-chloroethyl)-2-chloroethane-phosphonate, penta-bromo-diphenyl ether, tetrabromo-bis-phenol A, 1,2,3,4-tetrabromobutane, trimethyl phosphite, bromophthalic acid anhydride and brominated paraffins.

The water repellent agent may be, for example, methylhydrogen polysiloxane and dimethyl polysiloxane diol. The soil proof agent may be, for example, Scotchgard (trade name of a fluorine-containing resin type soil proof agent made by Minnesota Mining & Manufacturing Co., U.S.A.). The heat proof agent may be, for example, dimethyl polysiloxane diol and epoxy resin prepolymer. The antishrinking agent may be selected from dimethyl polysiloxane diol, reactive polyethylene and urethane prepolymer.

The wall constituent of the microcapsule may be composed of synthetic resin selected from polyurethanes, silicone resins, polyolefins, epoxy resins, polyamides, and polyesters.

The polyurethane resin for the wall constituent may be selected from toluylene diisocyanate, dimethyl diisocyanate, hexamethylene diisocyanate, xylene diisocyanate, methyl cyclohexane diisocyanate, triphenyl methane diisocyanate, diphenyl methane diisocyanate, and polymers prepared through reacting of polyurethane prepolymer having two or more isocyanate terminal groups with a polyvalent amine such as ethylene diamine, hexamethylene diamine, triethyl tetramine, paraphenylenediamine and piperazine, or with a polyvalent hydroxide compound such as 1,5-dihydroxy naphthalene, pyrogallol, 1,4-butadiene diol, glycerin, resorcin, bisphenol A.

The silicone resin may be prepared from organosiloxane prepolymer containing a main chain of polysiloxane of the formulas:



or



wherein R, R', R'' and R''' represent, for example, alkyl, 1,1,1-trifluoro propyl, cyanopolylalkyl, isocyanate, hydroxyl, methoxyl groups, same as or different from each other. The organosiloxane prepolymer preferably has a degree of polymerization of 2,000 or less so as to dissolve into hydrophobic solvent.

The epoxy resin may be produced from epoxy compounds to which are added polyvalent amine.

The polyester may be prepared, for example, by reacting a halide of polycarboxylic acid such as phthaloyl chloride, 1,4-cyclohexane dicarbonyl chloride, phosgene, 4,4'-biphenyl dicarbonyl chloride, adipoyl dichloride, sebacoyl chloride and terephthaloyl chloride with a phenolic compound such as resorcin, bisphenol A, 1,5-dihydroxy naphthalene, pyrogallol, phenolphthalein and primary condensation products of phenol resin.

10 The polyamide may be formed by reacting, for example, a halide of polycarboxylic acid such as sebacoyl chloride, 4,4'-biphenyl dicarbonyl chloride, phosgene, terephthaloyl dichloride, isophthaloyl dichloride, 1,4-cyclohexane dicarbonyl chloride and adipoyl dichloride with a polyamine such as ethylene diamine, hexamethylene diamine, triethylamine, tetramine, para-phenylene diamine and piperazine.

The reactive polyolefin derivative has a reactive radical such as chlorosulfonyl or acid chloride radical.

20 20 The polyolefin derivative containing the chlorosulfonyl radical is prepared by reacting polyethylene with chlorine and sulfuric acid gases. The chlorine atoms in the compound are effective to restriction of stereospecific property of the polyethylene chain and control of crystallization of the chain, in order to form a flexible polymer. In the chlorosulfonated polyethylene, the chlorine atoms are contained in primary or secondary form, and the chlorosulfonyl radical exist in primary, secondary or tertiary form and form a film by salt forming, cross-linking or sulfonic acid-linking with a compound having active hydrogen atom. Additionally, the chlorine atom existing at  $\beta$ -position of the chlorosulfonyl radical has chemical activity.

25 25 To improve the stability of the microcapsules in water, it is desirable that the wall constituent made up of the reactive polyolefin derivatives has a high elasticity. In order to meet the requirement, it is required that the derivative contains 25 to 30 percent by weight of chlorine and 1.5 percent by weight of sulphur, in other words, one atom of chlorine per 7 atoms of carbon and one unit of chlorosulfonyl group per 90 atoms of carbon.

30 30 The reactive polyolefin derivatives containing, as the reactive group, acid chloride group are prepared by reacting, for example, homo-polymer or copolymer of olefin derivatives having carboxylic group with phosphorous pentachloride. Such derivatives contains at least 0.1 percent by mol of acid chloride group and at least 50 percent by mol of olefin group.

35 35 The polymer containing the carboxylic group suitable for preparing the reactive polyolefin derivative containing the acid chloride group may be selected from, for example, ethylene-acrylic acid copolymer, ethylene-methacrylic acid copolymer, ethylene-itaconic acid copolymer, ethylene-methyl-hydrogen maleate copolymer, ethylene-

40 40 maleic acid copolymer, ethylene-acrylic acid-methyl methacrylate copolymer, ethylene-methacrylic acid-ethyl acrylate copolymer, ethylene-itaconic acid-methyl methacrylate copolymer, ethylene-methyl-hydrogen maleate-ethyl acrylate copolymer, ethylene-

45 45 methacrylic acid-vinyl acetate-copolymer, ethylene-acrylic acid-vinyl formate copolymer, ethylene-propylene-acrylic acid copolymer, ethylene-styrene-acrylic acid copolymer, ethylene-methacrylic acid-acrylonitrile copolymer, ethylene-fumaric acid-vinyl methyl ether copolymer, ethylene-vinyl chloride-acrylic acid copolymer, ethylene-vinyl-idenone chloride-acrylic acid copolymer, ethylene-vinyl fluoridemetha-

50 50

55 55

60 60

crylic acid polymer, ethylene-chlorotrifluoroethylene-methacrylic acid copolymer, polyethylene grafted by acrylic acid, polyethylene grafted by methacrylic acid, ethylene-propylene copolymer grafted by acrylic acid, ethylene-butene-1 copolymer grafted by methacrylic acid, ethylene-vinyl acetate copolymer grafted by methacrylic acid, polypropylene grafted by acrylic acid, polypropylene grafted by methacrylic acid, polybutene grafted by acrylic acid, poly-3-methyl butene grafted by acrylic acid and polyethylene grafted by acrylic acid and methyl acrylate. These polyolefin derivatives having the acid chloride group as the reactive group have a higher activity than that of the polyolefin derivatives having the chlorosulfonyl group, and thus the derivatives having the acid chloride group can self-cross link at low temperature. This point is valuable for preparing the microcapsules of the present invention. Further, it is more effective for accelerating the forming of the core constituent that 5 to 50 percent, preferably 10 to 20 percent by weight of active hydrogen-containing compound is added into the polymerization system.

The active hydrogen-containing compound may be selected from compound containing amino, imino, hydroxyl, carboxyl, or epoxy radical, particularly, benzidine, 4-4'-methylene bis-O-chloroaniline, 3'-3-dichlorobenzidine, hexamethylene diamine, 1,3-diamino propane, 1,2-diamino propane, and piperazine.

The wall constituent of the microcapsules may be composed of a synthetic resin shell formed by reaction between a prepolymer different from the hydrophobic treating agent and a hardening agent. Also, the wall constituent may be formed by interfacial polycondensation of the hydrophobic treating agent with a hardening agent or dispersing medium. For example, the wall constituent is formed from urethane prepolymer by interfacial polycondensation of the urethane prepolymer dispersed in water or an aqueous solution containing amine compound at interfaces between the dispersed particles and the dispersing medium.

According to the present invention, the solvent for the hydrophobic treating agent may be selected from non-aqueous solvents which are never mixcible with the dispersing medium and never swell or dissolve the synthetic resinous wall constituent. The solvent may be selected from tetrachloromethane, tetrachloroethylene, trichloroethylene, xylene, toluene, 1,1,1-trichloroethane, benzene, ethyl benzene, industrial gasoline, chloroform, methylenechloride, tetrachloroethane, tetrachlorodichloroethane and mixtures thereof.

In the preparation of the microcapsules of the present invention, the hydrophobic treating agent for the fibrous article and the polymerizing compound for forming the wall constituent are used at a ratio of 100:1 to 10,000:1. The non-aqueous solvent solution containing the treating agent and the polymerizing compound is finely dispersed in an aqueous dispersing medium into particles having a size of at most 100  $\mu\text{m}$ , and then the polymerizing compound interfacially forms a polymer at interfaces between the dispersed particles and the dispersing medium.

Preferably, the polymerizing compound is selected from urethane prepolymer having at least two -NCO group at molecular terminals thereof, polyorganosiloxane diol, polysulfide prepolymer, epoxy resin obtained

through reaction between bisphenol A and epichlorohydrin, and reactive polyolefin derivative having a reactive group such as an acid chloride or thionyl chloride group.

- 5 As stated hereinbefore, the proportion by weight of chloride wall constituent with respect to the core constituent is in a range from 1 : 500 to 1 : 5,000. If the proportion is lower than 1 : 10,000, the resultant wall constituent is insufficient due to too thin a thickness  
10 and a very low tenacity. If the proportion is higher than 1 : 100, the tenacity of the resultant wall constituent is too high for breakage thereof and it is very difficult to remove the broken wall constituent from the applied fibrous article. In view of this, the proportion of the  
15 wall constituent with respect to the core constituent must be in the abovementioned range. Only in this proportion, the microcapsules having the tenacity at break of at most 50 g/cm<sup>2</sup> can be obtained. Only such microcapsules can be industrially applied to the fibrous article  
20 at favorable conditions. In order to finely and uniformly disperse the nonaqueous solvent solution, it is preferable that the proportion by weight of the nonaqueous solvent solution with respect to the dispersing medium is at least 1 : 5, more preferably 1 : 1 to 1 : 3.  
25 Further, it is desirable for the above purpose that dispersing medium contains a proper dispersing agent.  
When the non-aqueous solvent solution of the treating agent has a low viscosity and is enclosed into the wall constituent by the above-mentioned process, the  
30 resultant microcapsules are desirable. However, when the non-aqueous solution has a high viscosity, it is very difficult to obtain the microcapsules having a thin wall constituent which is suitable for easily breaking at a small breaking force and high stability. That is, in the  
35 dispersing of the non-aqueous solvent solution, if the viscosity of the dispersed solution is too different from that of the dispersing medium, it is very difficult to form the dispersed solution into very fine and stable particles. Therefore, the proportion between these viscosities is preferably at most 1 : 5, more preferably 1 : 1 to 1 : 3.  
40

lose and carboxymethyl cellulose. Particularly, sodium alginate is most preferable for the process preparation of the microcapsules of the present invention due to its easy removing property from the surfaces of the resultant microcapsules by water rinsing.

The size of individual microcapsules produced in the polymerization system depends upon the size of the dispersed particles in the aqueous dispersing medium. In order to finely disperse the non-aqueous solvent solution, the mixture of the non-aqueous solvent solution and the aqueous dispersing medium is vigorously stirred with a stirrer such as a screw type, friction type, spiral type and homomixer type stirrers at for example, 8,000 or more rotations per minute into very fine particles of 30  $\mu\text{m}$  or a lesser size. Generally, when the stirrer is driven at 200 r.p.m. or less, the resultant microcapsules tend to have a size of 500  $\mu\text{m}$  or more. However, in the treatment of the fibrous articles, when the size of the microcapsules is too large, the size distribution is uneven and after the microcapsules applied to the fibrous article have been broken, it is difficult to remove the wall constituent residues from the fibrous article. Further, in this case, the impregnation of the fibrous article with the treating agent become uneven. Therefore, it is desirable that the size of the microcapsules is 100  $\mu\text{m}$  or less, more preferably 30  $\mu\text{m}$  or less. Accordingly, the velocity of stirring for the dispersion is preferably 200 r.p.m. or more, more preferably, 8,000 r.p.m. or more. Further, it is possible to easily obtain the superfine microcapsules of 5  $\mu\text{m}$  size or less through supplementarily utilizing an ultrasonic stirrer together with the usual stirrer.

The microcapsules of the present invention may be applied to the fibrous article in various manners such as blowing or electrostatic application of the dry microcapsules and padding or spraying application of an aqueous suspension of the microcapsules. The applied microcapsules are broken on the fibrous article by a suitable means such as a pressing roller mangle so as to impregnate the fibrous article with the content solution of the core constituents. Sometimes, the microcapsules may be broken by heating them to a temperature higher than the melting point of the wall constituent. The impregnated fabric may be heat-treated at a high temperature so as to fix the treating agent.

In this treatment of the fibrous article, it is desirable that the microcapsules are applied in an amount of 5 to 400 percent, more preferably, 10 to 100 percent based on the weight of the fibrous article. Also, it is allowed that two or more kinds of microcapsules which contain treating agents different from each other are applied to the fibrous article sometime within the process.

In order to break the microcapsules applied to the fibrous article, generally, the fibrous article is pressed with press rollers, squeezing rollers or a mangle at a pressure of 0.1 to 3 kg/cm<sup>2</sup>. If necessary, the fabric is subjected to heat treating at a temperature of 5° to 200°C for 10 seconds to 20 minutes, preferably, at 80° to 180°C temperature for 30 seconds to 5 minutes.

The individual microcapsule may contain two or more kinds of treating agents. The desired microcapsules may be mixed with other kinds of microcapsules at a desired proportion.

According to the present invention, the treating agent which needs a non-aqueous solvent can be easily applied to the fibrous article by utilizing the microcap-

sules in dry particulate form or aqueous suspension form.

Even if two kinds of treating agents are needed to treat the fibrous article being composed of two kinds of fibers or filaments and further, if the treating agents are insufficiently miscible with each other, it is possible that the fibrous article is treated with a mixture of two kinds of microcapsules each containing one kind of treating agent through one application.

Further, if the microcapsules are applied in aqueous suspension, it is possible that desired treating agents such as a moisture absorbing agent, softening agent, soil release agent, antistatic agent, dye and other hydrophilic treating agents are added into the aqueous suspension so that the fibrous article is treated with the microcapsules together with the added treating agent.

For example, the microcapsules containing a crease proof agent are suspended in an aqueous solution containing a moisture absorbing agent and the resultant

suspension is applied to the fibrous article. The moisture absorbing agent may be selected from compounds prepared by addition of 2 to 50 mol of ethylene oxide or propylene oxide to  $\epsilon$ -caprolactam, compounds prepared by addition of 2 to 50 mol of ethylene oxide or propylene oxide to  $\epsilon$ -caprolactam aligomer (dimer or trimer), sodium N-acylamino acetate, sodium N-acyl- $\alpha$ -amino propionate and sodium N-acyl- $\beta$ -amino propionate.

The applied fibrous article passes through a pair of rollers in order to squeeze excess suspension and break the microcapsules so as to impregnate the fibrous article with the non-aqueous solvent solution of the crease proof agent flowed out from the broken microcapsules.

At the same time, the fibrous article is impregnated with the moisture absorbing agent. Needless to say, the moisture absorbing agent may be contained in microcapsules if it is soluble in the non-aqueous solvent. Also, the moisture absorbing agent may be previously applied to the fibrous article before the application of the microcapsules. However, the aqueous solution of the moisture absorbing agent is effective for suspending the microcapsules in a favorable condition and the resultant fibrous article from the aqueous suspension has a superior crease recovery and durability. In view of this, the suspension containing the microcapsules and the moisture absorbing agent is preferably used at a high economical advantage. The above-stated advantage is caused from the fact that in microscopic view, the crease-proof agent flowed out from the broken microcapsules is unevenly or discontinuously distributed in the fibrous article and thus the moisture absorbing agent is distributed at portions not or insufficiently occupied by the crease proof agent.

Due to the uneven or complicated distribution of the crease-proof agent and the moisture absorbing agent, the treated fibrous article obtains the superior crease recovery property and moisture absorbing property.

However, the complicated distribution of two or more treating agents on the fibrous article are never found in the conventional application in which the treating agents are dissolved, emulsified or suspended into a bath together.

Furthermore, in order to obtain the preferable distribution of the treating agents, it is necessary that the non-aqueous solvent solution of the treating agent flowed out from the broken microcapsules does not diffuse to too wide a region. Accordingly, the non-

aqueous solvent solution of the treating agent should have pertinent viscosity, diffusing coefficient and contact angle. In consideration of this, in order to achieve satisfactory crease-proof and moisture absorbing properties on the fibrous article the size of the microcapsule should be in a range of at most 500 $\mu$ m, preferably at most 100 $\mu$ m and more preferably at most 30 $\mu$ m. In this case, the size of the microcapsules less than 1 $\mu$ m is undesirable because of the lowering effect of the complicated distribution.

The non-aqueous solvent solution of the crease-proof agent preferably has a viscosity of up to 2,000 cp, more preferably, 10 to 1,000 cp in order to have a pertinent diffusion property in the fibrous article and to keep the effect of the moisture absorbing agent. In view of this, urethane prepolymer, as a crease-proof agent, should be dissolved into a content of 5 to 60 percent by weight, preferably 20 to 50 percent by weight, acrylic resin prepolymer 1 to 70, preferably 5 to 50 percent by weight and silicone resin prepolymer 5 to 100, preferably, 15 to 100 percent by weight depending on its molecular weight.

The application quantity of the microcapsules may be regulated depending on the kind of the fibrous article, kind, viscosity and concentration of the treating agent and size of the microcapsules used.

From our experiments, a proportion of the total area occupied by the microcapsules distributed on the fibrous article with respect to the area of the fibrous article is preferably 1 : 2 to 1 : 50, more preferably 1 : 4 to 1 : 30. If the proportion exceeds 1 : 2, the moisture absorbing property of the resultant fibrous article is unsatisfactory and if the proportion is less than 1 : 50, the crease recovery is unsatisfactory. Actually, the content of the microcapsules in the aqueous suspension is preferably in a range from 2 to 10 percent by weight.

The fibrous fabric treated through the above-stated process is impregnated with 0.3 to 6.0 percent by weight of the creaseproof agent distributed discontinuously and 0.1 to 5.0 percent preferably 0.2 to 3.0 by weight of the moisture absorbing agent continuously distributed at portions between the portions occupied by the crease-proof agent.

In each treatment, the crease-proof agent contained in the microcapsules may be a mixture of two or more compounds and a mixture of two or more kinds of microcapsules each containing a crease-proof agent different from each other may be used.

The fibrous article usable for the present invention may be optionally selected from yarns, knitted fabrics, woven fabrics, non-woven fabrics and these laminates made up of natural fibers or filaments such as wool, silk, cotton, ramie and linen and artificial fiber or filaments such as polyamide polyester polyacrylic polymeric, polyvinyl alcohol, polyolefin, polyvinyl chloride, polyvinyl chloridene and polyurea fiber or filaments, rayon and acetate fibers or filaments.

The process of the present invention has the following advantages.

1. The treatment can be carried out in an open apparatus although a non-aqueous volatile solvent is used, because the volatile solvent is enclosed in the microcapsules.

2. The treating agent dissolved in the volatile solvent can be maintained for a long period of time.

3. The application of the microcapsules of the present invention has the similar effect as that of the conventional manner in which the non-aqueous solution of the treating agent is applied to the fibrous article.

4. The microcapsules have uniform size and are easily broken due to their very low tenacity.

10 5. Color of the microcapsules never changes with lapse of time, for example, days.

6. The wall constituent residues of the broken microcapsules are not found on the treated fibrous article according to naked eye observation due to their very thin thickness.

15 7. The wall constituent is fused at the heat-treating temperature and effects on the fibrous article to improve its treating effect and durability.

20

### EXAMPLE 1

#### Microcapsules Containing a Silicone Type Elasticity Improving Agent

25 5 g of resorcin were dissolved in 400 cc of an aqueous solution containing 1 percent of sodium hydroxide. 0.2 g of toluylene diisocyanate, 20 g of organopolysiloxane diol prepolymer having a degree polymerization of 300 and 0.02 g of di-N-butyl-tin-dilauroate were dissolved in

30 200 g of trichloroethylene. The trichloroethylene solution was slowly dropped into the aqueous solution at room temperature stirring with a stirrer at 800 r.p.m. in order to disperse the trichloroethylene solution into very fine particles.

35 After 1 hour, numerous microcapsules were formed. These composition and features were as indicated in Table 1.

40

Table 1

| Composition                                  | Core constituent | Trichloroethylene solution of organopolysiloxane prepolymer |
|----------------------------------------------|------------------|-------------------------------------------------------------|
|                                              | Wall constituent | Polyurethane                                                |
| Ratio by weight of wall with respect to core |                  | 1:1,000                                                     |
| Tenacity at break                            |                  | 10 g/cm <sup>2</sup>                                        |
| Size                                         |                  | 20 - 30 $\mu$ m                                             |

50

The microcapsules prepared thus were distributed on an acrylic twill fabric to a content of 100 percent based on the weight of the fabric. The fabric was pressed by a pair of rubber rollers having a hardness of 60 at a pressure of 1.0 kg/cm<sup>2</sup> in order to break the microcapsules. Through the press, the fabric was substantially evenly impregnated with the core constituent solution of the microcapsules and the wall constituent residues remained on the periphery surface of the press roller.

55 60 The fabric was dried at 80°C temperature and then heat-treated at 120°C temperature for 5 minutes. The resultant fabric had a preferable hand feeling and excellent compression elasticity and crease recovery as shown in Table 2.

65

Table 2

| Item             | Compressive Elasticity (%) |            | Crease Recovery |      | Hand                               |
|------------------|----------------------------|------------|-----------------|------|------------------------------------|
|                  | Percentage                 | Elasticity | Warp            | Weft |                                    |
| Fabric           |                            |            |                 |      | Feeling                            |
| Treated fabric   | 21.8                       | 91.8       | 90.5            | 9.5  | Highly rigid and resilient         |
| Untreated fabric | 20.5                       | 83.8       | 83.2            | 87.3 | Insufficiently rigid and resilient |

Note: \*1 Compressive elasticity was determined by the following manner. Four pieces of fabric to be tested are superimposed and compressed at a weight of  $10 \text{ g/cm}^2$  for 1 minute into a thickness of  $t$ . Then, the compressed testing pieces are further compressed at a weight of  $300 \text{ g/cm}^2$  for 1 minute into a thickness of  $t_1$  followed by releasing the compression for 1 minute into a thickness of  $t_2$ . Percentage compression and elasticity are given by the following equations:

$$\text{Percentage compression} = \frac{t - t_1}{t} \times 100$$

$$\text{Compressive elasticity} = \frac{t_2 - t_1}{t - t_1} \times 100$$

\*2 Crease recovery was determined through JIS L-1079, 5-22-2, B-method.

### EXAMPLE 2

#### Microcapsules Containing a Flame-Proof Agent

5 g of bis-phenol A was dissolved in 200 cc of an aqueous solution containing 1 percent sodium hydroxide.

1,200 g of a tetrachloroethylene solution containing 0.4 g of hexamethylene diisocyanate and 10 g of (a flame proof agent) was slowly dropped into the aqueous solution stirring with a stirrer at 400 r.p.m. at room temperature in order to disperse the tetrachloroethylene solution into very fine particles. After stirring for 1 hour, numerous microcapsules having a composition and features as indicated in Table 3 were obtained.

Table 3

| Composition                     | Core constituent | Tetrachloroethylene solution of Unflame 3BP |  |
|---------------------------------|------------------|---------------------------------------------|--|
|                                 | Wall constituent | Polyurethane                                |  |
| Ratio by weight of wall to core |                  | 1:3,000                                     |  |
| Tenacity at break               |                  | 10 g/cm <sup>2</sup>                        |  |
| Size                            |                  | 200 - 400 $\mu\text{m}$                     |  |

The microcapsules were uniformly applied to a polyethylene terephthalate broad cloth to a content of 70 percent based on the weight of the cloth and then pressed with a pair of rubber rollers having a hardness of 70 at a pressure of  $1.0 \text{ kg/cm}^2$ . The cloth was uniformly impregnated with the core constituent solution flowing out from the broken microcapsules. The cloth was dried at  $70^\circ\text{C}$  temperature followed by heat-treating at  $160^\circ\text{C}$  temperature for 30 seconds. The resultant treated cloth had an excellent flame proof property as illustrated in Table 4

Table 4

| Item            | Flame Proof Property |                  |
|-----------------|----------------------|------------------|
|                 | Before laundering    | After laundering |
| Fabric          |                      |                  |
| Treated cloth   | 5                    | 4                |
| Untreated cloth | 1                    | 1                |

Laundering was carried out using an aqueous solution of 1 g of Zabu (trade name of a detergent made by Kao Sekken Kabushiki Kaisha, Japan) in 1 l of water at a liquor ratio of 1 : 50 at  $40^\circ\text{C}$  temperature for 60 minutes.

### EXAMPLE 3

#### Microcapsules Containing an Antistatic Agent

4 g of resorcin and 1 g of 1,5-dihydroxy naphthalene were dissolved in 200 cc of an aqueous solution of 2 percent sodium hydroxide. Into the aqueous solution, 90 g of a 1,1,1-tri-chloroethane solution containing 0.15 g of diphenylmethane diisocyanate and 5 g of an antistatic agent was slowly dropped with stirring by a stirrer at 600 r.p.m. at room temperature in order to disperse the 1,1,1-trichloroethane solution into very fine particles.

After the 1,1,1-trichloroethane solution was uniformly dispersed, the temperature of the system was raised to  $50^\circ\text{C}$  and maintained at this temperature for 2 hours with stirring. The result was numerous microcapsules having the composition and properties as illustrated in Table 5.

Table 5

| Composition                     | Core constituent | 1,1,1-trichloroethane solution containing antistatic agent |
|---------------------------------|------------------|------------------------------------------------------------|
|                                 | Wall constituent | Polyurethane                                               |
| Ratio by weight of wall to core |                  | 1:600                                                      |
| Tenacity at break               |                  | 15 g/cm <sup>2</sup>                                       |
| Size                            |                  | 50 - 60 $\mu\text{m}$                                      |

The resultant microcapsules were applied to a polycapramide tricot fabric and the fabric was pressed according to the same method as that of Example 1. The fabric was air dried and then heat-treated at  $160^\circ\text{C}$  temperature for 1 minute. The resultant fabric had excellent antistatic property and durability as illustrated in Table 6.

Table 6

| Item             | Frictional static voltage (volt) *4 |                  |
|------------------|-------------------------------------|------------------|
|                  | Before laundering                   | After laundering |
| Treated fabric   | 120                                 | 3,500            |
| Untreated fabric | 12,000                              | 10,500           |

Note: \*4 Frictional static voltage was determined by means of a rotary static tester made by Kowa Shokai, Japan, using a friction element consisting of 60° cotton broad cloth.

### EXAMPLE 4

#### Microcapsules Containing Water Repellent Agent

4 g of resorcin was dissolved into 200 cc of an aqueous solution containing 0.8% by weight of sodium hydroxide and 105 g of a tetrachloroethylene solution containing 0.07 g of hexamethylene diisocyanate, 5 g of methyl-hydrogen-polysiloxane prepolymer having a degree of polymerization of 20, 1 g of dimethyl polysiloxane diol prepolymer having a degree of polymerization of 300 and 0.08 g of n-dibutyl tin dilaurate was prepared. The tetrachloroethylene solution was slowly dropped into the aqueous solution at room temperature stirring with a stirrer at 900 r.p.m. in order to disperse the tetrachloroethylene solution into very fine particles. After the uniform dispersion was completed, the system was heated to a temperature of 40°C and remained at this temperature for 1 hour while stirring. The result was microcapsules having a composition and properties as illustrated in Table 7.

Table 7

|                                 |                  |                                                                                                                            |
|---------------------------------|------------------|----------------------------------------------------------------------------------------------------------------------------|
| Composition                     | Core constituent | Tetrachloroethylene solution containing methyl hydroxide polysiloxane prepolymer and dimethyl polysiloxane diol prepolymer |
|                                 | Wall constituent | Polyurethane                                                                                                               |
| Ratio by weight of wall to core |                  | 1:1,500                                                                                                                    |
| Tenacity at break               |                  | 11 g/cm <sup>2</sup>                                                                                                       |
| Size                            |                  | 20 - 30 $\mu$ m                                                                                                            |

According to the same method as that indicated in Example 1, a broad cloth consisting of 65 percent by weight of polyethylene terephthalate fiber and 35 percent by weight of cotton fiber was impregnated with the above-prepared microcapsules and then pressed in order to break the microcapsules. The treated broad cloth was dried at 60°C temperature followed by heat-treatment at 160°C temperature for 3 minutes. The resultant fabric had a preferable hand feeling and an excellent waterrepellent properties as illustrated in Table 8.

Table 8

| Fabric           | Water-repellent property *5 |                  |                            |
|------------------|-----------------------------|------------------|----------------------------|
|                  | Before laundering           | After laundering | Hand feeling               |
| Treated fabric   | 100                         | 100              | Elegantly soft & resilient |
| Untreated fabric | 30                          | 30               | Un-satisfactory            |

Note: \*5 Water repellent property was determined by AATCC, 22-1952, spray method.

### EXAMPLE 5

#### Microcapsules Containing Oil Repellent Agent

6.0 g of bisphenol A was dissolved in 240 cc of an aqueous solution of 1 percent sodium hydroxide. Also, 0.1 g of hexamethylene diisocyanate and 10 g of Scotchgard FC-310 (trade name of an oil repellent agent made by Minnesota Mining & Manufacturing Co., U.S.A.) were dissolved into 120 g of 1,1,1-trichloroethane. The trichloroethane solution was slowly dropped into the aqueous solution stirring with a stirrer at 11,000 r.p.m. in order to disperse the trichloroethane solution into very fine particles. The dispersion was heated to 50°C and maintained at this temper-

ature with stirring. The result was microcapsules having the composition and properties as indicated in Table 9.

TABLE 9

| Composition | Core constituent                | Solution of Scotchgard FC-310 in 1,1,1-trichloroethane |
|-------------|---------------------------------|--------------------------------------------------------|
|             | Wall constituent                | Polyurethane                                           |
| 10          | Ratio by weight of wall to core | 1:1,200                                                |
|             | Tenacity at break               | 22 g/cm <sup>2</sup>                                   |
|             | Size                            | 5 - 10 $\mu$ m                                         |

15

- The microcapsules prepared thus were applied to a double interlock knitted fabric made up of worsted yarns and then broken in the same manner as that of Example 2. The fabric was impregnated with Scotchgard flowing out from the broken microcapsules. The impregnated fabric was dried at 40°C temperature and then heat-treated at 140°C temperature for 3 minutes. For comparison, the same fabric as that of the present Example was impregnated with a solution of Scotchgard FC-310 in 1,1,1-trichloroethane at an impregnating quantity of 3.0 percent based on the weight of the fabric. The results of the present and comparison Examples had oil and water repellent properties as shown in Table 10.

Table 10

| Fabric | Item               | Oil repellent property *6 |                  | Water repellent property |                  |
|--------|--------------------|---------------------------|------------------|--------------------------|------------------|
|        |                    | Before laundering         | After laundering | Before laundering        | After laundering |
| 40     | Example 5          | 76                        | 72               | 98                       | 95               |
|        | Comparison Example | 76                        | 72               | 98                       | 96               |

Note: \*6 Oil repellent property was determined by AATCC, 118-1966 T.

45

The laundering was carried out by the manner as indicated in Example 2.

Table 10 shows the fact that the treated fabric of the present invention has excellent oil and water repellent properties similar to that of the comparison Example which of course is normal for Scotchgard 310.

### EXAMPLE 6

#### Microcapsule Containing a Flame Proof Agent

20 g of 2,3-dibromopropyl phosphate, 0.2 g of dimethyl polysiloxane diol having a degree of polymerization of 500 and 0.4 g of n-dibutyl tin dilaurate were dissolved in 400 g of trichloroethylene. The solution was slowly dropped into 2,000 cc of water with stirring at 6,500 r.p.m. at room temperature so as to form numerous very fine dispersed particles of the solution. The dispersion was heated to 60°C and maintained at this temperature for 1 hour while stirring. The result was microcapsules having the composition and properties as indicated in Table 11.

Table 11

|                                 |                                                                    |
|---------------------------------|--------------------------------------------------------------------|
| Core constituent                | Solution of tris-2,3-dibromo-propyl phosphate in trichloroethylene |
| Composition                     |                                                                    |
| Wall constituent                | Silicone resin                                                     |
| Ratio by weight of wall to core | 1:2,000                                                            |
| Tenacity at break               | 5 g/cm <sup>2</sup>                                                |
| Size                            | 40 - 50 µm                                                         |

The microcapsules was applied to a polyethylene terephthalate broad cloth to a content of 80 percent based on the weight of the fabric followed by breaking them by pressing at a pressure of 1.2 kg/cm<sup>2</sup> with a pair of rubber rollers having a hardness of 60.

The fabric was uniformly impregnated with the flame proof agent flowing out from the broken microcapsules. The impregnated fabric was dried at 70°C temperature and then heat-treated at 160°C temperature for 30 seconds. The resultant fabric had an excellent flame proof property before and after laundering as indicated in Table 12. Laundering was performed by the manner as indicated in Example 1.

Table 12

| Item             | Flame proof property |                  |
|------------------|----------------------|------------------|
|                  | Before laundering    | After laundering |
| Fabric           |                      |                  |
| Treated fabric   | 5                    | 4                |
| Untreated fabric | 1                    | 1                |

## EXAMPLE 7

## Microcapsules Containing an Antistatic Agent

A solution of 5 g of antistatic agent, 1.0 g of diethyl polysiloxane diol and 0.1 g of stannous octoate in 800 g tetrachloroethylene was slowly dropped into 4,000 of an aqueous solution containing 1 percent by weight of sodium alginate stirring at 4,000 r.p.m. at room temperature so as to disperse the tetrachloroethylene solution into very fine particles. The dispersion was maintained for 2 hours, while stirring. The result was numerous microcapsules having the composition and properties as illustrated in Table 13.

Table 13

|                                 |                  |                                                     |
|---------------------------------|------------------|-----------------------------------------------------|
| Composition                     | Core constituent | Solution of antistatic agent in tetrachloroethylene |
|                                 | Wall constituent | Silicone resin                                      |
| Ratio by weight of wall to core |                  | 1:800                                               |
| Tenacity at break               |                  | 20 g/cm <sup>2</sup>                                |
| Size                            |                  | 60 - 70 µm                                          |

The microcapsules prepared thus was applied to a polycapramide tricot fabric to a content of 100 percent based on the weight of the fabric followed by breaking them by pressing with a pair of rubber rollers having 70 hardness at a pressure of 1.5 kg/cm<sup>2</sup>.

The fabric was uniformly impregnated with the anti-static agent flowing out from the broken microcapsules. The impregnated fabric was air dried and then heat-treated at 160°C for 1 minute. The resultant fabric

had a superior antistatic property as shown in Table 14.

Table 14

| Item             | Frictional static voltage (volt) |                  |
|------------------|----------------------------------|------------------|
|                  | Before laundering                | After laundering |
| Fabric           |                                  |                  |
| Treated fabric   | 100                              | 3,500            |
| Untreated fabric | 12,000                           | 10,500           |

10

## EXAMPLE 8

## Microcapsules Containing Oil Repellent Agent

A solution containing 10 g of Scotchgard FC-310, 0.5 g of dimethyl polysiloxane diol having a degree of polymerization of 800 and 0.2 g of n-dibutyl tin succinate in 500 g of tetrachloroethylene was dispersed into 3,000 cc of an aqueous solution containing 0.3 percent by weight of dispersing agent by stirring at 11,000 r.p.m. at room temperature. After stirring for 3 hours, the dispersion resulted in microcapsules suspended in the aqueous solution. The microcapsules prepared thus had the composition and property as indicated in Table 15.

25

Table 15

|                                 |                  |                                                   |
|---------------------------------|------------------|---------------------------------------------------|
| Composition                     | Core constituent | Solution of Scotchgard 310 in tetrachloroethylene |
|                                 | Wall constituent | Silicone resin                                    |
| Ratio by weight of wall to core |                  | 1:1,000                                           |
| Tenacity at break               |                  | 10 g/cm <sup>2</sup>                              |
| Size                            |                  | 10 - 30 µm                                        |

35

The microcapsules were applied to a double interlock knitted worsted fabric and broken in the same manner as that of Example 6.

The fabric impregnated with the oil repellent agent was dried at 40°C temperature and then heat-treated at 140°C temperature for 3 minutes. The result had superior oil and water repellent properties as shown in Table 16.

45

Table 16

| Item               | Water repellent property |                  | Oil repellent property |                  |
|--------------------|--------------------------|------------------|------------------------|------------------|
|                    | Before laundering        | After laundering | Before laundering      | After laundering |
| Fabric             |                          |                  |                        |                  |
| Example 8          | 75                       | 70               | 96                     | 95               |
| Comparison Example | 76                       | 72               | 98                     | 96               |

55 The comparison Example was carried out in the same manner indicated in Example 5.

Table 16 shows the fact that the oil repellent fabric of the present invention had superior oil and water repellent properties similar to that of the comparison Example in which Scotchgard 311 was applied to the fabric in a standard manner.

## EXAMPLE 9

## Microcapsules Containing a Dye

60 A solution of 0.5 g of a disperse dye, 0.5 g of methylphenyl polysiloxane diol and 0.1 g of n-dibutyl tin diocylate in 1,000 g of trichloroethylene was dispersed into 5,000 cc of an aqueous solution containing 0.2 percent

by weight of carboxymethyl cellulose of 40°C temperature by slowly dropping while vigorously stirring at 12,000 r.p.m. The dispersion was heated to 60°C and maintained at this temperature for 1 hour while stirring. The dispersion formed numerous microcapsules having the composition and properties as shown in Table 17.

Table 17

|                                 |                  |                                               |
|---------------------------------|------------------|-----------------------------------------------|
| Composition                     | Core constituent | Solution of disperse dye in trichloroethylene |
|                                 | Wall constituent | Silicone resin                                |
| Ratio by weight of wall to core |                  | 1:2,000                                       |
| Tenacity at break               |                  | 8 g/cm <sup>2</sup>                           |
| Size                            |                  | 5 - 10 µm                                     |

In accordance with the manner indicated in Example 6, the microcapsules were applied to a tricot fabric consisting of diacetate fibers and then broken in order to impregnate the fabric with the dye solution. The fabric was dried at 60°C temperature and then heat-treated at 170°C temperature for 1 minute. The resultant fabric had been dyed deep blue.

## EXAMPLE 10

Microcapsules Containing an Ultra-Violet Ray Absorber

A solution of 0.5 g of 2-hydroxy-4-octoxy benzophenone, 1 g of methyl-hydrogen-polysiloxane and 0.1 g of stannous Octoate in 800 g of 1,1,1-trichloroethane was dispersed into 4,000 cc of water by slowly being dropped at room temperature while vigorously stirring at 6,000 r.p.m. The dispersion was heated to 40°C and maintained at this temperature for 2 hours while stirring. The dispersion was converted to microcapsules having the composition and properties as shown in Table 18.

Table 18

|                                 |                  |                                                                     |
|---------------------------------|------------------|---------------------------------------------------------------------|
| Composition                     | Core constituent | Solution of 2-hydroxy-4-octoxybenzophenone in 1,1,1-trichloroethane |
|                                 | Wall constituent | Silicone resin                                                      |
| Ratio by weight of wall to core |                  | 1:800                                                               |
| Tenacity at break               |                  | 15 g/cm <sup>2</sup>                                                |
| Size                            |                  | 50 - 60 µm                                                          |

In accordance with the same manner as that of Example 6, the microcapsules were applied to fine polycapramide taffeta fabrics which were dyed various colors with acid or disperse dyes indicated in Table 19 and then broken on the fabrics. The dyed fabrics impregnated with the ultra-violet ray absorber was air dried and then heat-treated at 150°C temperature for 2 hours. The resultant dyed fabrics had a superior light fastness higher than that of the untreated fabrics and comparison treated fabrics which were treated with a benzene solution of the ultra-violet ray absorber. The results were shown in Table 19.

Table 19

| 5  | Item                             | Percent of fading of dyed fabric irradiated by Fade-O-meter for 20 hours |                  |                |
|----|----------------------------------|--------------------------------------------------------------------------|------------------|----------------|
|    |                                  | Fabric                                                                   | Untreated fabric | Treated fabric |
| 10 | Dye *6 and concentration %       |                                                                          |                  |                |
|    | Supranol Brilliant Red 6BW 1%    | 30                                                                       | 5                | 5              |
|    | Xylene Fast Blue BL 1.5%         | 40                                                                       | 15               | 10             |
|    | Kiton Green V 2.0%               | 90                                                                       | 60               | 60             |
| 15 | Resoline Brilliant Blue PBB 0.3% | 50                                                                       | 20               | 12             |
|    | Diacelliton Brown G 0.5%         | 60                                                                       | 20               | 20             |

Note: \*6 Supranol Brilliant Red 6BW is trade name of an acid dye (C.I. Acid Violet 97) made by Bayer, Germany. Xylene Fast Blue BL is trade name of an acid dye (C.I. Acid Blue 59) made by Sandoz, Switzerland. Kiton Green V is trade name of an acid dye (C.I. 440250) made by Ciba, Switzerland. Resoline Brilliant Blue PBB is trade name of a disperse dye made by Bayer, Germany. Diacelliton Brown G is trade name of a disperse dye made by Mitsubishi Kasei, Japan.

Table 19 shows the facts that the treated fabrics of the present Example had a light fastness higher than that of the untreated fabrics, respectively, and that the light fastness of the treated fabrics of the present Example is similar to those of the comparison fabrics which were treated by the conventional manner.

## EXAMPLE 11

Treatment of a Jersey Fabric Consisting of False Twisted Textured Polycapramide Yarns for Improving Its Elasticity

1. The preparation of microcapsules containing an elasticity improving agent  
0.75 of dimethyl polysiloxane diol prepolymer having a degree of polymerization of 800, 0.1 g of a polyurethane prepolymer and 0.01 g of di-n-butyl tin dilaurate were dissolved into 50 g of trichloroethylene. The trichloroethylene solution was dispersed into 600 cc of aqueous solution containing 1 g of dispersing agent by slowly dropping while stirring at 8,000 r.p.m. After the dropping had been completed, the stirring was continued for 10 minutes. 30 cc of an aqueous solution containing 10 percent by weight of ethylene diamine based on the total weight of the solution were dropped into the dispersion while stirring and then stirred for 30 minutes at room temperature. Through the procedure, the urethane prepolymer having diisocyanate residue was reacted with ethylene diamine at interfaces between water and the dispersed fine particles of the trichloroethylene solution so as to produce solid polymer which forms the wall constituents of the microcapsules. The resultant microcapsules contained trichloroethylene solution of dimethyl polysiloxane diol prepolymer and di-n-butyl tin dilaurate as the core constituent.

The microcapsules were recovered through precipitation water-rinsing and filtration.

The resultant microcapsules had the composition and properties as indicated in Table 20.

Table 20

|                                 |                                                                                                                                          |
|---------------------------------|------------------------------------------------------------------------------------------------------------------------------------------|
| Core constituent                | Solution of 1.5% by weight of dimethyl-polysiloxane diol prepolymer and 0.02% by weight of di-n-butyl tin dilaurate in trichloroethylene |
| Composition                     |                                                                                                                                          |
| Wall constituent                | Polyurethane                                                                                                                             |
| Ratio by weight of wall to core | 1:500                                                                                                                                    |
| Tenacity at break               | 12 g/cm <sup>2</sup>                                                                                                                     |
| Size                            | 20 - 30 $\mu$ m                                                                                                                          |

## 2. Treatment of the fabric

The microcapsules prepared thus were uniformly applied to a triple interlock jersey fabric prepared from false twisted textured polycapramide yarns of 70 deniers/18 filaments/2P, to a content of 110 percent based on the weight of the fabric. The fabric was pressed with a pair of rubber rollers having a hardness of 60° at a pressure of 1.5 kg/cm<sup>2</sup> in order to break the microcapsules. The wall constituents of the broken microcapsules maintained on the peripheral surface of the roller and the core constituent flowed out from the broken microcapsules and impregnated the fabric. The impregnated fabric was dried at 80°C and heat-treated at 150°C for 3 minutes. The treated fabric contained 1.6 percent organopolysiloxane based on the weight of the fabric and had the properties as shown in Table 21.

Table 21

| Item              | Tensile Elasticity   |                | Compressive Elasticity |            |
|-------------------|----------------------|----------------|------------------------|------------|
|                   | Load for stretch (g) | Elasticity (%) | Compressive ratio      | Elasticity |
| Untreated fabric  | 15.0                 | 80.3           | 18.8                   | 71.0       |
| Treated fabric    | 12.0                 | 93.6           | 19.8                   | 94.3       |
| Comparison fabric | 12.0                 | 94.0           | 20.6                   | 94.3       |

The comparison fabric was prepared by impregnating the same fabric as that of the present Example with 1.6 percent of organopolysiloxane based on the weight of the fabric and then heat-treating the impregnated fabric.

## EXAMPLE 12

### Shrink-Proof Treatment of Worsted Jersey Fabric

#### 1. Preparation of microcapsules

0.15 g of Zeset T (trade name of a reactive polyethylene type shrink proofing agent for wool fiber made by Du Pont, U.S.A.) and 0.2 g of hexamethylene diisocyanate were dissolved into 100 cc of tetrachloroethylene. The solution was slowly dropped into 170 cc of an aqueous solution containing 4 g of bisphenol A and 1 percent by weight of potassium hydroxide while stirring at 6,500 r.p.m. so as to disperse the tetrachloroethylene solution into very fine particles. Through this procedure, the hexamethylene diisocyanate reacted with the bisphenol A at interfaces between water and the dispersed particles of the tetrachloroethylene so as to produce a solid polymer forming the wall constituents of numerous microcapsules which contained the core constituent.

The microcapsules prepared thus had the composition and properties as shown in Table 22.

Table 22

|    |                                 |                  |                                            |
|----|---------------------------------|------------------|--------------------------------------------|
| 5  | Composition                     | Core constituent | Solution of Zeset T in tetrachloroethylene |
|    |                                 | Wall constituent | Polyurethane                               |
| 10 | Ratio by weight of wall to core |                  | 1:800                                      |
|    | Tenacity at break               |                  | 12 g/cm <sup>2</sup>                       |
|    | Size                            |                  | 30 - 50 $\mu$ m                            |

## 2. Treatment of fabric

The microcapsules were uniformly applied to a double interlock jersey fabric consisting of 1/44° worsted 15 yarns to a content of 80 percent based on the weight of the fabric. The fabric was pressed with a pair of rubber rollers having a hardness of 40 at a pressure of 1.0 kg/cm<sup>2</sup> in order to break the microcapsules. The wall constituents of the broken microcapsules remained on 20 the peripheral surface of the rollers and the content solution of the core constituent evenly penetrated into the fabric. The fabric was dried at 70°C temperature followed by heat treating at 130°C temperature for 1.5 minutes.

25 The resultant fabric contained 2.4 percent of the shrink proof agent based on the weight of the fabric, and had a shrinkage as shown in Table 23. For comparison, the same fabric as that of the present Example was impregnated with tetrachloroethylene solution of Zeset 30 T to a content of 2.4 percent based on the weight of the fabric and treated in the same manner as stated above.

Table 23

| 35                | Item   | Shrinkage in area (%)        |                             |
|-------------------|--------|------------------------------|-----------------------------|
|                   |        | After one time of laundering | After five times laundering |
| 35                | Fabric |                              |                             |
| Untreated fabric  |        | 30                           | 40                          |
| Treated fabric    |        | 10                           | 12                          |
| Comparison fabric |        | 9                            | 12                          |

45 Table 23 shows the fact that the fabric treated in the present Example had superior shrink proof properties similar to that of the comparison fabric which was treated by the conventional manner.

## EXAMPLE 13

### Crease Proof and Water Repellent Treatment for a Polyethylene Terephthalate Fiber/Cotton Blend Fabric

#### 1. Preparation of microcapsules containing crease proof and water repellent agents

50 4 g of methyl-hydrogen polysiloxane prepolymer having a degree of polymerization of 20, 1 g of dimethyl polysiloxane diol prepolymer, 0.06 g of stannous octoate and 0.2 g of Epikote 828 (trade name of an epoxy resin made by Shell Oil Co., U.S.A.) were dissolved 55 into 100 cc of 1,1,1-trichloroethane. The solution was dispersed into 600 cc of an aqueous solution containing 1 g of dispersing agent by slowly dropping while stirring at 8,000 r.p.m. After the dispersing was completed, 10 cc of a solution of an amine type hardening agent T (trade name of a hardening agent for epoxy resin made by Shell Oil Co.) was dropped into the dispersion. The dispersion was heated to 40°C temperature. Through 60 the procedure, Epikote 828 was hardened by action of the hardening agent T at interfaces between water and the dispersed fine particles of 1,1,1-trichloroethane 65

into solid polymer forming the wall constituents of the microcapsules which contains 1,1,1-trichloroethane solution of methyl hydrogen polysiloxane prepolymer, dimethyl polysiloxane diol prepolymer and stannous octoate. The resultant microcapsules had the composition and properties as shown in Table 24.

Table 24

|                                 |                  |                                                                                                                                          |
|---------------------------------|------------------|------------------------------------------------------------------------------------------------------------------------------------------|
| Composition                     | Core constituent | Solution of methyl hydrogen polysiloxane prepolymer, dimethyl polysiloxane diol prepolymer and stannous octoate in 1,1,1-trichloroethane |
|                                 | Wall constituent | Epoxy resin                                                                                                                              |
| Ratio by weight of wall to core |                  | 1:800                                                                                                                                    |
| Tenacity at break               |                  | 10 g/cm <sup>2</sup>                                                                                                                     |
| Size                            |                  | 20 - 30 $\mu$ m                                                                                                                          |

## 2. Treatment of fabric

The microcapsules suspended in water were applied to a broad cloth consisting of polyethylene terephthalate fiber/cotton (65 : 35 by weight) blend yarns to a content of 130 percent based on the weight of the fabric. The fabric was dried at 100°C temperature and pressed with a pair of a rubber rollers having a hardness of 40 at a pressure of 1.0 kg/cm<sup>2</sup> so as to break the microcapsules. The wall constituents of the broken microcapsules remained on the peripheral surface of the press roller and the core constituent flowed out onto the fabric so as to uniformly impregnate the fabric. The impregnated fabric was dried at 60°C temperature followed by heat-treating at 130°C temperature for 3 minutes.

The treated fabric contained 1.2 percent organo polysiloxane based on the weight of the fabric and had the superior crease recovery and water repellent property as shown in Table 25. For comparison, a same fabric as that of the present Example was impregnated with the 1,1,1-trichloroethane solution of the same treating agents as those of the present Example so that the content of the organo polysiloxane produced on the fabric was 1.2 percent based on the weight of the fabric, and dried followed by heat-treating at the same temperatures as those of the present Example.

Table 25

| Fabric            | Crease recovery (%) |               |                       |                       |                          |
|-------------------|---------------------|---------------|-----------------------|-----------------------|--------------------------|
|                   | Original Warp       | Original Weft | After laundering Warp | After laundering Weft | Water repellent property |
| Untreated fabric  | 80.0                | 78.8          | 78.8                  | 74.4                  | 30                       |
| Treated fabric    | 85.6                | 82.5          | 83.6                  | 81.6                  | 100                      |
| Comparison fabric | 85.6                | 82.7          | 83.5                  | 81.8                  | 100                      |

Table 25 shows the fact that the treated fabric had a crease recovery and water repellent property similar to the comparison fabric which was treated in the conventional manner.

## EXAMPLE 14

### Treatment for Light-Fade Proofing of Dyed Fabric

#### 1. Preparation of microcapsules

1 g of 2-hydroxy-4-octoxy benzophenone and 0.1 g of terephthaloyl chloride were dissolved in 100 g of benzene. The solution was uniformly dispersed in 1,200

cc of an aqueous solution containing 1.0 g of hexamethylene diamine by slowly dropping while stirring at 4,800 r.p.m. After the dispersion was maintained at room temperature from 2 hours, a solid polymer was produced at interfaces between water and the dispersed particles of the benzene solution so as to form numerous microparticle wall constituents.

The microcapsules thus obtained had the composition and properties as illustrated in Table 26.

Table 26

|                                 |                  |                                                        |
|---------------------------------|------------------|--------------------------------------------------------|
| Composition                     | Core constituent | Solution of 2-hydroxy-4-octoxy benzophenone in benzene |
|                                 | Wall constituent | Polyamide                                              |
| Ratio by weight of wall to core |                  | 1:500                                                  |
| Tenacity at break               |                  | 7 g/cm <sup>2</sup>                                    |
| Size                            |                  | 40 - 60 $\mu$ m                                        |

## 2. Treatment of fabric

The microcapsules were applied to fine polycapramide taffeta fabrics dyed with various disperse or acid dyes to a content of 50 percent based on the weight of the fabric in such a static electrical manner that the microcapsules were distributed on the fabric by brushing through a metallic mesh plate between which and an electrode facing the mesh plate, a voltage of 1,000 to 12,000 volts was applied. The fabric was pressed with a metallic roller at a pressure of 1.0 kg/cm<sup>2</sup> in order to break the microcapsules. Through this procedure, the fabric was uniformly impregnated with the core constituent solution flowing out from the broken microcapsules. The fabric was dried at 120°C temperature for 1 minute.

The treated fabric had superior fade proof properties as shown in Table 27. For comparison, the same fabric as that of the present Example was impregnated with the benzene solution of 2-hydroxy-4-octoxy benzophenone the same as that of the present Example and dried at 120°C temperature for 1 minute.

Table 27

| Item                             | Percent of fading of dyed fabric irradiated by Fade-O-meter for 20 hours |                  |                |
|----------------------------------|--------------------------------------------------------------------------|------------------|----------------|
|                                  | Fabric                                                                   | Untreated fabric | Treated fabric |
| Dye and concentration (% o.w.f.) |                                                                          |                  |                |
| Supranol Brilliant Red 6BW 1%    | 30                                                                       | 5                | 5              |
| Xylene Fast Blue BL 1.5%         | 40                                                                       | 15               | 10             |
| Kiton Green V 2.0%               | 90                                                                       | 60               | 60             |
| Resoline Brilliant Pink PBB 0.3% | 50                                                                       | 10               | 12             |
| Diacelliton Brown G S/F 0.5%     | 60                                                                       | 20               | 20             |

As is clearly shown in Table 27, the treated fabric of the present Example had an improved high fastness.

## EXAMPLE 15

Flame Proof Treatment of Lace Curtain Made Up of 20 percent by Weight of Polyethylene Terephthalate Filament and 20 percent by Weight of Rayon Filament

#### 1. Preparation of microcapsules A

15 g of Bigol 40BXE (trade name of a halogenated organic phosphorous compound type flame proof agent made by Daikyo Kagaku Kabushiki Kaisha, Japan) and 0.1 g of Desmodur L (trade name of an urethane prepolymer made by Bayer, Germany) were dissolved in 85 g of toluene. The solution was dispersed in 1,000 cc of an aqueous solution containing 1 g of dispersing agent by slowly dropping while stirring at 6,500 r.p.m. After the dropping had been completed, the stirring was maintained for 30 minutes and then 10 cc of an aqueous solution containing 10 percent by weight of ethylene diamine was added so as to form numerous microcapsules A from Desmodur L. The resultant microcapsules A had the composition and properties as shown in Table 28.

Table 28

| Composition                     | Core constituent | Solution of 15% by weight of Bigol 40BXE in toluene |
|---------------------------------|------------------|-----------------------------------------------------|
|                                 | Wall constituent | Polyurethane                                        |
| Ratio by weight of wall to core |                  | 1:1,000                                             |
| Tenacity at break               |                  | 7 g/cm <sup>2</sup>                                 |
| Size                            |                  | 40 - 50 µm                                          |

### 2. Preparation of microcapsules B

10 g of Flame Proof MC (trade name of a polyammonium phosphate type flame proof agent made by Nihon Senka Kabushiki Keisha, Japan) and 0.5 g of hexamethylene diamine were dissolved in 90 g of water. The aqueous solution was dispersed in 800 g of trichloroethylene solution containing 0.3 g of Desmodur L by dropping slowly while vigorously stirring at 6,500 r.p.m. After the dropping was completed, the stirring was continued for 30 minutes so as to produce a solid polymer for forming the wall constituent of the microcapsules at interfaces between the trichloroethylene solution and the dispersed particles of the aqueous solution. The resultant microcapsules B had the composition and properties as shown in Table 29.

Table 29

| Composition                     | Core constituent | Solution of 10% by weight of Flame Proof MC in water |
|---------------------------------|------------------|------------------------------------------------------|
|                                 | Wall constituent | Polyurethane                                         |
| Ratio by weight of wall to core |                  | 1:1,000                                              |
| Tenacity at break               |                  | 10 g/cm <sup>2</sup>                                 |
| Size                            |                  | 40 - 60 µm                                           |

### 3. Treatment of fabric

An aqueous suspension containing the microcapsules A and the microcapsules B in a proportion of 1 to 1 was sprayed onto the lace curtain which consisted of 20 percent by weight of rayon filaments located at edge portions of the curtain and 80 percent by weight of polyethylene terephthalate located at ground portion thereof and having a weight of 750 g/m<sup>2</sup>. The sprayed fabric contained 15 percent of the microcapsules A and 15 percent of the microcapsules B based on the weight of the fabric. The fabric was dried at 50°C temperature and then pressed with a mangle having a hardness of 70 at a pressure of 1.3 kg/cm<sup>2</sup> so as to break the applied microcapsules. Through this procedure, the fabric was uniformly impregnated with the flame proof agents

flowing out from the broken microcapsules. The fabric was heat-treated at 150°C temperature for 3 minutes. Whereas Bigol 40BXE is effective for flame proofing the polyethylene terephthalate fibers and Flame Proof MC is effective for rayon fibers, they cannot be dissolved in each other. Therefore, in the conventional method, these flame proof agents cannot be used together. However, the method of the present invention can resolve the difficulty. The resultant fabric had a superior flame proof property as shown in Table 30. For comparison, the same lace curtain as that of the present Example was treated in such a manner that firstly, the fabric was impregnated with an aqueous emulsion containing Bigol 40BXE at a pickup of 50 percent and then dried followed by heat-treating at 150°C temperature and secondly, the fabric was further impregnated with an aqueous solution of Flame Proof MC at a pick-up of 50 percent and then dried followed by heat-treating.

Table 30

| Fabric            | Item | Flame Proof Property       |                  |                                                        |
|-------------------|------|----------------------------|------------------|--------------------------------------------------------|
|                   |      | Polyethylene terephthalate |                  |                                                        |
|                   |      | Original                   | After laundering | Rayon                                                  |
| Untreated fabric  |      | 1                          | 1                | Burnt                                                  |
| Treated fabric    |      | 6                          | 5                | Non-burnt but fall due to melting of polyester portion |
| Comparison fabric |      | 6                          | 5                |                                                        |

Table 30 clearly shows the fact that the fabric treated by one spray in accordance with the method of the present invention had a superior flame proof properties same as that of the comparison fabric which was treated through two padding operations.

### EXAMPLE 16

#### 40 Treatment for Improving Elasticity and Antipilling Property of Acrylic Fabric

##### 1. Preparation of microcapsules

3.5 g of urethane prepolymer containing 3 percent of -NCO group and 0.5 g of Desmodur L was dissolved in 50 g of trichloroethylene. The solution was dispersed into 1,000 cc of an aqueous solution containing 1 percent by weight of sodium alginate by slowly dropping while stirring at 6,500 r.p.m. at room temperature. After stirring for 20 minutes, 20 cc of an alkaline solution containing 10 percent by weight of bis-phenol A was added to the dispersion and then the dispersion was heated to 30°C temperature for 30 minutes. Through the procedure, numerous microcapsules were obtained. The resultant microcapsules had the composition and properties as shown in Table 31.

Table 31

| Composition                     | Core constituent | Solution of urethane polymer in trichloroethylene |
|---------------------------------|------------------|---------------------------------------------------|
|                                 | Wall constituent | Polyurethane                                      |
| Ratio by weight of wall to core |                  | 1:1,200                                           |
| Tenacity at break               |                  | 8 g/cm <sup>2</sup>                               |
| Size                            |                  | 30 - 40 µm                                        |

##### 2. Treatment of fabric

The microcapsules prepared thus was applied to a twill fabric made up of Cashimilon fibers (trade name of an acrylic fiber made by Asahi Kasei Kabushiki Kaisha, Japan) so as to contain 100 percent of the microcapsules based on the weight of the fabric and in accordance with the manner indicated in Example 11. The fabric was pressed in the same method as stated in Example 11. The pressed fabric was dried at 50°C temperature and then heat-treated at 120°C temperature for 5 minutes. The resultant fabric contained 1.6 percent of polyurethane based on the weight of the fabric and had the superior properties as shown in Table 32.

Table 32

| Item              | Compressive elasticity |                | Crease recovery (original) (%) |      | Fabric | Original | After laundering | Original | After laundering | depth (K/S) *7 |
|-------------------|------------------------|----------------|--------------------------------|------|--------|----------|------------------|----------|------------------|----------------|
|                   | Percentage (%)         | Elasticity (%) | Warp                           | Weft |        |          |                  |          |                  |                |
| Untreated fabric  | 20.5                   | 83.8           | 85.5                           | 87.3 |        |          |                  |          |                  |                |
| Treated fabric    | 23.0                   | 90.0           | 90.2                           | 93.2 |        |          |                  |          |                  |                |
| Comparison fabric | 22.8                   | 90.2           | 89.9                           | 93.1 |        |          |                  |          |                  |                |

## EXAMPLE 17

Treatment for Coloring and Water and Oil Proofing Acetate Fabric

## 1. Preparation of microcapsules

In accordance with the same process as indicated in Example 11, numerous microcapsules containing a solution of Scotchgard FC-310 and Foron Red FL (trade name of a disperse dye made by Sandoz, Switzerland) were prepared. The resultant microcapsules had the composition and properties as shown in Table 33.

Table 32

| Item              | Compressive elasticity |                | Crease recovery (original) (%) |      | Fabric | Original | After laundering | Original | After laundering | depth (K/S) *7 |
|-------------------|------------------------|----------------|--------------------------------|------|--------|----------|------------------|----------|------------------|----------------|
|                   | Percentage (%)         | Elasticity (%) | Warp                           | Weft |        |          |                  |          |                  |                |
| Untreated fabric  | 20.5                   | 83.8           | 85.5                           | 87.3 |        |          |                  |          |                  |                |
| Treated fabric    | 23.0                   | 90.0           | 90.2                           | 93.2 |        |          |                  |          |                  |                |
| Comparison fabric | 22.8                   | 90.2           | 89.9                           | 93.1 |        |          |                  |          |                  |                |

## 2. Treatment of fabric

The resultant microcapsules were applied to a tricot fabric made up of diacetate filaments and the fabric was pressed in accordance with the same method as stated in Example 11. The fabric was dried at 60°C

temperature and then heat-treated at 170°C temperature for 1 minute.

The resultant fabric was colored red and had superior oil and water repellent properties as shown in Table 34.

Table 34

| Item              | Oil repellent property |          | Water repellent property |          | Color            |  |
|-------------------|------------------------|----------|--------------------------|----------|------------------|--|
|                   | Fabric                 | Original | After laundering         | Original | After laundering |  |
| Treated fabric    | 95                     | 95       | 75                       | 70       | 12.2             |  |
| Comparison fabric | 98                     | 95       | 75                       | 70       | 11.0             |  |

Note: \*7 Color depth was determined in accordance with Kubelka Munks' equation:

$$K/S = \frac{(1 - R)^2}{2R}$$

where R is the reflectance of monochromatic light from an infinitely thick pad of the fabric, K is the absorption coefficient of the fabric, and S is the scattering coefficient. For comparison, the same fabric as that of the present Example was treated by the same solution as that contained in the microcapsules of the present Example.

Table 34 clearly shows that the dyed fabric of the present Example had superior oil and water repellent properties and color depth similar to those of the comparison fabric which was treated by the conventional method.

## EXAMPLE 18

## Dyeing of Cotton Fabric

## 1. Preparation of microcapsules

Microcapsules A containing a benzene solution of cyanuric chloride were prepared by the process as stated in Example 11, and microcapsules B containing an aqueous solution of Eriochrome Brown BR (trade name of an acid mordant dye made by Geigy, Switzerland C.I. 11290) were prepared by the process as indicated in Example 15. These microcapsules A and B had the compositions and properties as shown in Table 35.

Table 35

| Item                            | Microcapsules                                                    |                  | A                                                        | B          |
|---------------------------------|------------------------------------------------------------------|------------------|----------------------------------------------------------|------------|
|                                 | Core constituent                                                 | Wall constituent |                                                          |            |
| Composition                     | Solution containing 3% by weight of cyanuric chloride in benzene | Polyurethane     | Aqueous solution of 2% by weight 30 μEriochrome Brown BR |            |
| Ratio by weight of wall to core |                                                                  | 1:200            |                                                          | 1:200      |
| Tenacity at break               |                                                                  | 15 g/cm²         |                                                          | 16 g/cm²   |
| Size                            |                                                                  | 40 - 50 μm       |                                                          | 20 - 30 μm |

## 2. Treatment of fabric

The resultant microcapsules A and B were applied to a 60 s' cotton broad cloth by the static electrical method as indicated in Example 14 so that the micro-

capsules A and B were contained in the fabric at a content of 50 percent based on the weight of the fabric, respectively. The fabric was pressed in accordance with the method of Example 14 and dried at 100°C temperature followed by heat-treating at 150°C temperature for 3 minutes. The result is indicated in Table 36. For comparison, the same fabric as that of the present Example was treated only by the content solution of the micro-capsules B (Comparison fabric A) and then half of the treated fabric was treated by the content solution of the microcapsules A (Comparison fabric B).

Table 36

| Fabric                        | Item               | Colorfastness for washing |
|-------------------------------|--------------------|---------------------------|
| Comparison fabric A           | Removed by washing |                           |
| Comparison fabric B           | Washable brown     |                           |
| Fabric of the present Example | Washable brown     |                           |

## EXAMPLE 19

0.3 g of ethylene-vinyl acetate-methacryloyl chloride (70/24/6) copolymer, 30 g of organo polysiloxane prepolymer and 0.3 g of Catalyst for polymerizing silicone resin and 0.06 g of a hardening agent dissolved in 169 g of tetrachloroethylene. The solution was dispersed into 1,000 cc of an aqueous solution containing 0.2 percent by weight of hydroxyethyl cellulose by slowly dropping while vigorously stirring at 8,000 r.p.m. at room temperature. Through stirring for 1 hour, numerous microcapsules were formed. The resultant microcapsules had the composition and properties as shown in Table 37.

Table 37

|                                 |                  |                                                                   |
|---------------------------------|------------------|-------------------------------------------------------------------|
| Composition                     | Core constituent | Solution of organo polysiloxane prepolymer in Tetrachloroethylene |
|                                 | Wall constituent | Ethylene-vinyl acetate-methacryloyl chloride copolymer            |
| Ratio by weight of wall to core |                  | 1:500                                                             |
| Tenacity at break               |                  | 12 g/cm <sup>2</sup>                                              |
| Size                            |                  | 20 - 30 $\mu$ m                                                   |

The microcapsules were uniformly applied to a twill fabric made up of Toraylon fibers (trade name of an acrylic fiber made by Toray Industries Inc., Japan) to a content of 100 percent based on the weight of the fabric, and the fabric was pressed with a pair of rubber rollers having a hardness of 70 at a pressure of 1.2 kg/cm<sup>2</sup>. Through breaking the microcapsules, while the fabric was uniformly impregnated with the content solution of the microcapsules, the broken core constituents were not formed on the fabric according to the naked eye. The impregnated fabric was dried at 80°C temperature and then heat-treated at 120°C temperature for 5 minutes. The resultant fabric had superior elasticity and crease recovery and preferable hand feeling as shown in Table 38.

Table 38

| 5                | Fabric | Compressive elasticity (%) |            | Crease recovery (%) |      | Hand feeling   |
|------------------|--------|----------------------------|------------|---------------------|------|----------------|
|                  |        | Percent compression        | Elasticity | Warp                | Weft |                |
| Untreated fabric |        | 20.5                       | 83.8       | 83.2                | 87.3 | Low Resilient  |
| Treated fabric   |        | 22.9                       | 93.0       | 91.5                | 92.6 | High resilient |

## EXAMPLE 20

15 0.2 g of ethylene-methacryl chloride (97/3) copolymer and 20 g of tris-2,3-dibromopropyl phosphate were dissolved in 8.8 g of toluene. The solution was dispersed in 1,000 cc of an aqueous solution containing 0.5 percent by weight of sodium alginate by slowly dropping at room temperature while stirring at 7,200 r.p.m. The dispersion was heated to 80°C temperature and maintained at this temperature for 40 minutes. Numerous microcapsules having the composition and properties as shown in Table 39 were obtained.

Table 39

| 30                              | Composition | Core constituent | Solution of tris-2,3-dibromopropyl phosphate in toluene |
|---------------------------------|-------------|------------------|---------------------------------------------------------|
|                                 |             | Wall constituent | Ethylene-methacryl chloride copolymer                   |
| Ratio by weight of wall to core |             |                  | 1:600                                                   |
| Tenacity at break               |             |                  | 11 g/cm <sup>2</sup>                                    |
| Size                            |             |                  | 30 - 40 $\mu$ m                                         |

40 The microcapsules prepared thus were applied to a broad cloth consisting of polyethylene terephthalate yarns to a content of 80 percent based on the weight of the fabric. The fabric was pressed in the same manner as indicated in Example 11. The fabric was impregnated with the core constituent solution. The impregnated fabric was dried at 50°C temperature and then heat-treated at 150°C temperature for 2 minutes. The resultant fabric contained 15.5 percent by weight of tris-2,3-dibromopropyl phosphate as a flame proof agent and had superior flame resisting properties. The wall constituents of the broken microcapsules were not found on the pressed fabric according to the naked eye.

45 For comparison, the same fabric as that of the present Example was treated with the same solution as contained in the microcapsules of the present Example by the padding manner so as to pick up 15.5 percent of the flame proof agent based on the weight of the fabric.

50 The results are shown in Table 40.

Table 40

| 60                | Fabric | Flame proof property |                  |
|-------------------|--------|----------------------|------------------|
|                   |        | Original             | After laundering |
| Untreated fabric  |        | 1                    | 1                |
| Treated fabric    |        | 5                    | 4                |
| Comparison fabric |        | 5                    | 4                |

65 Table 40 shows the fact that the treated fabric of the present Example had a superior flame proof property and high durability similar to those of the comparison

fabric which was treated by the conventional method.

### EXAMPLE 21

A solution in 98 g of 1,1,1-trichloroethane was prepared from 0.07 g of chlorosulfonated polyethylene of the formula:



and 2 g of Teracyl Navy Blue RL (trade name of a disperse dye made by Ciba, Switzerland) and 0.01 g of hardening agent. The solution was dispersed in 700 cc of an aqueous solution containing 1% by weight of a dispersing agent by slowly dropping at room temperature while vigorously stirring at 5,000 r.p.m. The dispersion was heated to 50°C temperature and maintained at this temperature for 1 hour while stirring. Numerous microcapsules having the composition and properties as shown in Table 41 were prepared.

Table 41

|                                    |                                      |                                                                                               |
|------------------------------------|--------------------------------------|-----------------------------------------------------------------------------------------------|
| Composition                        | Core constituent<br>Wall constituent | Solution of Teracyl Navy Blue<br>RL in 1,1,1-trichloroethane<br>Chlorosulfonated polyethylene |
| Ratio by weight of wall<br>to core |                                      | 1:1,500                                                                                       |
| Tenacity at break                  |                                      | 5 g/cm <sup>2</sup>                                                                           |
| Size                               |                                      | 5 - 10 $\mu$ m                                                                                |

The microcapsules prepared thus were uniformly applied to a tricot fabric made up of diacetate filament in the same manner as indicated in Example 11 to a content of 50 percent based on the weight of the fabric. The fabric impregnated with the core constituent solution of the microcapsules was air dried and then heat-treated at 160°C temperature for 5 minutes. The resultant fabric was colored deep blue and its colorfastness and color tone were similar to those of the fabric dyed in an aqueous dyeing bath by the conventional method.

**EXAMPLE 22**

0.1 g of ethylene-methacryl chloride (84/16) copolymer and 1 g of 2-hydroxy-4-octoxy benzophenone were dissolved in 99g of tetrachloromethane. The solution was finely dispersed into 1,000 cc of an aqueous solution containing 1 g of dispersing agent by slowly dropping at room temperature while vigorously stirring at 7,500 r.p.m. The dispersion was heated to 40°C temperature and maintained at this temperature while stirring for 30 minutes. Thus, numerous microcapsules having the composition and properties as shown in Table 42 were obtained.

Table 42

|                                 |                  |                                                                   |
|---------------------------------|------------------|-------------------------------------------------------------------|
| Composition                     | Core constituent | Solution of 2-hydroxy-4-octoxy benzophenone in tetrachloromethane |
|                                 | Wall constituent | Ethylene-methacryl chloride copolymer                             |
| Ratio by weight of wall to core |                  | 1:1,000                                                           |
| Tenacity at break               |                  | 2 g/cm <sup>2</sup>                                               |
| Size                            |                  | 20 - 40 µm                                                        |

The microcapsules prepared thus were applied to several fabrics made up of polycapramide or polyethylene terephthalate fibers which fabrics have been dyed 5 with acid or disperse dye having a low light-fastness, respectively, to a content of 70 percent based on the weight of each fabric. These applications were carried out in the same manner as indicated in Example 11. 10 The fabrics impregnated with the core constituent solution containing 2-hydroxy-4-octoxy benzophenone which is an ultra-violet ray absorber were heat-treated at 170°C temperature for 2 minutes. The dyed fabrics treated thus had the improved light fastness as shown 15 in Table 43.

Table 43

|          |           | Percent of fading of dyed fabric irradiated by<br>fade-O-meter for 20 hours                                                           |                          |                      |                    |
|----------|-----------|---------------------------------------------------------------------------------------------------------------------------------------|--------------------------|----------------------|--------------------|
|          |           | Dye and its<br>concentration<br>(% o.w.f.)                                                                                            | Un-<br>treated<br>fabric | Fabric               |                    |
|          |           |                                                                                                                                       | Treated<br>fabric        | Comparison<br>fabric |                    |
| Material |           |                                                                                                                                       |                          |                      |                    |
| 20       |           |                                                                                                                                       |                          |                      |                    |
| 25       | Polyamide | Supranol Brilliant Blue<br>6BW 1.0%<br>Kiton green V<br>2.0%<br>Resoline<br>Brilliant Pink<br>PBB 0.3%<br>Diacelliton<br>Green G 0.5% | 30<br>90<br>50<br>60     | 5<br>60<br>10<br>20  | 5<br>60<br>9<br>20 |
| 30       |           |                                                                                                                                       |                          |                      |                    |
| 35       | Polyester | Miketon Polyester Brown<br>2R 3.0%<br>Samaron Red<br>HF 3.0%                                                                          | 70<br>65                 | 20<br>10             | 20<br>10           |

0 Note: Diacelliton green G is trade name of a disperse dye made by Mitsubishi Kasei, Japan. Miketon Polyester Brown 2R is trade name of a disperse dye made by Mitsui Toatsu Kagaku, Japan. Samaron Red HF is trade name of a disperse dye made by Hoechst, Germany.

45 For comparison, the same fabrics as those of the present Examples were sprayed with the same solution as contained in the microcapsules of the present Examples.

Table 43 shows the fact that the dyed fabric treated in the present Example had improved high-fastnesses similar to those of the comparison fabrics.

### EXAMPLE 23

55 0.13 g of ethylene-methacryl chloride-vinyl acetate  
(80/5/15) copolymer 4 g of methyl-hydrogen  
polysiloxane prepolymer, 1 g of dimethyl polysiloxane  
diol prepolymer and 0.06 g of stannous octoate were  
dissolved into 95 g of tetrachloroethylene. The solution  
60 was finely dispersed into 500 cc of an aqueous solution  
containing 1.0 percent by weight of hydroxyethyl cellulose  
by slowly dropping at room temperature while stirring  
at 8,500 r.p.m. The dispersion was heated to 45°C  
temperature and maintained at this temperature while  
65 stirring for 1 hour. Thus, numerous microcapsules having  
the composition and properties as shown in Table  
44 were obtained.

Table 44

|                                 |                  |                                                                                                                      |
|---------------------------------|------------------|----------------------------------------------------------------------------------------------------------------------|
| Composition                     | Core constituent | Solution of methyl-hydrogen polysiloxane prepolymer and dimethyl polysiloxane diol prepolymer in tetrachloroethylene |
|                                 | Wall Constituent | Ethylene-methacryl chloride-vinyl acetate copolymer                                                                  |
| Ratio by weight of wall to core |                  | 1:800                                                                                                                |
| Tenacity at break               |                  | 7 g/cm <sup>2</sup>                                                                                                  |
| Size                            |                  | 10 - 30 $\mu$ m                                                                                                      |

The microcapsules prepared thus were uniformly applied to a broad cloth consisting of polyester fiber-cotton (65 : 35 by weight) blend yarns to a content of 110% based on the weight of the fabric. The application and the breaking of the microcapsules were performed in accordance with the same method as indicated in Example 11 except the hardness of the rubber rollers is 50. The fabric impregnated with the core constituent solution of the microcapsules which contained water repellent agents was dried at 100°C temperature and then heat-treated at 160°C temperature for 5 minutes. The resultant fabric had a superior water repellent property and a preferable hand feeling as illustrated in Table 45.

Table 45

| Fabric           | Item | Water repellent property (%) | Hand feeling       |
|------------------|------|------------------------------|--------------------|
| Treated fabric   |      | 100                          | soft and resilient |
| Untreated fabric |      | below 50                     | rigid              |

## EXAMPLE 24

40 parts of urethane prepolymer having a molecular weight of 18,000 and containing 1.8 percent by mol of  $-NCO$  group were dissolved in 60 parts of tetrachloroethylene. The urethane prepolymer was prepared from polypropylene glycol having a molecular weight of 2,000, tolylene diisocyanate and polypropylene triol. 200 g of this solution were dispersed in 600 g of an aqueous solution containing 0.85 percent by weight of sodium alginate by slowly dropping at room temperature for 15 minutes while stirring with a homomixer at 7,000 r.p.m. 45

After the dispersing was completed, 2 cc of an aqueous solution containing 10 percent by weight of ethylene diamine was added to the dispersion while stirring at 3,000 r.p.m. and then the dispersion was left to stand for 24 hours. Through this procedure, numerous microcapsules having the composition and properties as shown in Table 46. The obtained microcapsules were recovered from the dispersion by decantation, rinsed with water and then dried.

Table 46

|                                 |                  |                                                      |
|---------------------------------|------------------|------------------------------------------------------|
| Composition                     | Core constituent | Solution of urethane prepolymer in trichloroethylene |
|                                 | Wall constituent | Polyurethane                                         |
| Ratio by weight of wall to core |                  | 1:1,000                                              |

Table 46-Continued

|    |                   |                                                      |
|----|-------------------|------------------------------------------------------|
| 5  | Core constituent  | Solution of urethane prepolymer in trichloroethylene |
|    | Composition       | Polyurethane                                         |
| 10 | Tenacity at break | 5 g/cm <sup>2</sup><br>10-30 $\mu$ m                 |

An amount of the microcapsules having a total apparent volume of 100 ml were suspended in 2,000 cc of an aqueous solution containing 40 g of perspiration absorbing agent for fibrous articles so as to obtain a 15 treating suspension for fibrous articles.

The treating suspension was applied to a tricot fabric consisting of polycapramide filament yarn of 45 denier/7 filaments, and then the fabric was squeezed with a roller mangle having a hardness of 50 in the same 20 manner indicated in Example 11 in order to break temperature microcapsules. The fabric was dried at 100°C temperature and heat-treated at 130°C temperature for 3 minutes.

The resultant fabric had a superior crease recovery 25 and water absorbency as indicated in Table 47. For comparison, the same fabric as that of the present Example was treated only with the same solution as that contained in the microcapsules of the present Example.

30

Table 47

| 35                | Item   | Crease Recovery (%) |      |                  |              | Water-absorbency |                  |
|-------------------|--------|---------------------|------|------------------|--------------|------------------|------------------|
|                   |        | Original            |      | After laundering |              | (*) 8 (sec.)     |                  |
|                   | Fabric | Warp                | Weft | Warp             | Weft         | Original         | After laundering |
| Untreated fabric  | 71.1   | 95.5                | 64.8 | 95.1             | 52           | 15               |                  |
| Treated fabric    | 79.0   | 99.8                | 72.8 | 98.7             | 5.8          | 12               |                  |
| Comparison fabric | 80.0   | 100.0               | 74.0 | 99.3             | over 5 mins. | over 5 mins.     |                  |

Note: (\*) 8. Water-absorbency of fabric was determined in such a manner that 0.03 cc of an aqueous solution of 1% by weight of potassium permanganate were dropped down to a center of a circle of 3 cm diameter marked on the fabric to be tested, and then the time in second consumed for diffusing the dropped solution to the circle is determined.

50

## EXAMPLE 25

A trichloroethylene solution containing 100 parts of organo polysiloxane prepolymer, 1 part of Catalyst for polymerizing silicone resin, 1 part of Catalyst PD and 0.4 parts of the same urethane prepolymer as used in Example 24 was dispersed in an aqueous solution containing 5 percent by weight of hydroxyethyl cellulose in accordance with the method as indicated in Example 24.

The resultant microcapsules had the composition and 60 properties as indicated in Table 48.

Table 48

|                         |             |                  |                                                                               |
|-------------------------|-------------|------------------|-------------------------------------------------------------------------------|
| 65                      | Composition | Core constituent | Solution of organo polysiloxane prepolymer, and Catalyst in trichloroethylene |
|                         |             | Wall constituent | Polyurethane                                                                  |
| Ratio by weight of wall |             |                  |                                                                               |

Table 48-Continued

|                   |                  |                                                                               |
|-------------------|------------------|-------------------------------------------------------------------------------|
| Composition       | Core constituent | Solution of organo polysiloxane prepolymer, and Catalyst in trichloroethylene |
|                   | Wall constituent | Polyurethane                                                                  |
| to core           |                  | 1:800                                                                         |
| Tenacity at break |                  | 3 g/cm <sup>2</sup>                                                           |
| Size              |                  | 10 - 30 $\mu$ m                                                               |

An amount of the resultant microcapsules having a total apparent volume of 300 ml were suspended in 10 liters of aqueous solution containing 1 Kg of a perspiration absorbing agent.

The suspension was applied to a tricot fabric made up of polyethylene terephthalate filament yarn of 100 deniers/32 filaments and then the fabric was pressed in the same process as indicated in Example 24. The fabric was dried at 100°C temperature for 3 minutes and then heat-treated at 160°C temperature for 30 seconds.

The resultant fabric had superior crease recovery and water-absorbency as shown in Table 49. For comparison, the same fabric as that of the present Example was treated with the same solution as that contained in the microcapsules of the present Example.

Table 49

| Fabric             | Item         |              | Crease recovery (%) |                  | Water absorbency (second) |                  |
|--------------------|--------------|--------------|---------------------|------------------|---------------------------|------------------|
|                    | Warp         | Weft         | Original            | After laundering | Original                  | After laundering |
|                    |              |              | Warp                | Weft             |                           |                  |
| Untreated          | 55.0         | 82.5         | 55.1                | 80.5             | Over 5 mins.              | Over 5 mins.     |
| Treated Comparison | 85.1<br>86.2 | 90.6<br>91.8 | 83.0<br>83.1        | 89.2<br>90.2     | Over 5 mins.              | Over 5 mins.     |

## EXAMPLE 26

Microcapsules A were prepared from a solution of 5 parts of butyl acrylate-acrylonitrile-acrylic acid copolymer and 0.2 parts of urethane prepolymer containing 13.0 percent of -NCO group which was prepared from tolylene diisocyanate and trimethylol propane (3 : 1 by mol) in 94.8 parts of trichloroethylene, and an aqueous solution containing 7 percent by weight of a perspiration absorbing agent in the same manner as indicated in Example 24.

Microcapsules B were prepared from the same solutions and in the same method as those indicated in Example 24.

These microcapsules A and B had the composition and properties as shown in Table 50, respectively.

Table 50

| Item        | Microcapsule            | A                                                   | B                                                    |
|-------------|-------------------------|-----------------------------------------------------|------------------------------------------------------|
|             | Core constituent        | Solution of acrylic prepolymer in trichloroethylene | Solution of urethane prepolymer in trichloroethylene |
| Composition | Wall constituent        | Polyurethane                                        | Polyurethane                                         |
|             | Ratio by weight of wall |                                                     |                                                      |

Table 50-Continued

| Item              | Microcapsule        | A                                                   | B                                                    |
|-------------------|---------------------|-----------------------------------------------------|------------------------------------------------------|
|                   | Core constituent    | Solution of acrylic prepolymer in trichloroethylene | Solution of urethane prepolymer in trichloroethylene |
| Composition       | Wall constituent    | Polyurethane                                        | Polyurethane                                         |
|                   | to core             | 1:1,500                                             | 1:1,000                                              |
| Tenacity at break | 3 g/cm <sup>2</sup> | 2 g/cm <sup>2</sup>                                 |                                                      |
| Size              | 10-30 $\mu$ m       | 10-30 $\mu$ m                                       |                                                      |

15 500 ml apparent volume of the microcapsules A and 200 ml apparent volume of the microcapsules B were suspended in 5 litres of an aqueous solution containing 75 g of Lurotex A-25.

20 A tricot fabric consisting of polycapramide filament yarns of 45 deniers/10 filaments was impregnated with the suspension, squeezed, dried at 80°C temperature for 5 minutes and then heat-treated at 140°C temperature for 5 minutes. The resultant fabric had a superior crease recovery and water absorbency as shown in Table 51.

25 For comparison, the same fabric as that of the present Example was impregnated with the same solution as that contained in the microcapsules A and then with the same solution as that contained in the microcapsules B.

Table 51

| Fabric     | Item |      | Crease recovery (%) |       | Water absorbency (sec.) |              |
|------------|------|------|---------------------|-------|-------------------------|--------------|
|            | Warp | Weft | Original            | After | Original                | After        |
|            |      |      | Warp                | Weft  | laundering              | laundering   |
| Untreated  | 63.9 | 76.9 | 63.2                | 75.8  | 135                     | 60           |
| Treated    | 82.9 | 84.6 | 80.2                | 80.1  | 7                       | 13           |
| Comparison | 83.0 | 86.7 | 82.5                | 85.6  | Over 5 mins.            | Over 5 mins. |

## EXAMPLE 27

50 0.2 part of urethane prepolymer which was obtained from 1 mol of copolyester having a molecular weight of 2,000 and prepared from a mixture of butylene glycol and propylene glycol (90 : 10) and adipic acid, 4 mol of hexamethylene diisocyanate and 4 mol of 1,4 butane diol, 50 parts of organo polysiloxane prepolymer, 0.5 parts of Catalyst for polymerizing silicone resin, and 0.5 parts of Catalyst for polymerizing silicone resin were dissolved in 44.8 parts of trichloroethylene.

55 The solution was finely dispersed in an aqueous solution of 2.55 parts of sodium alginate in 300 parts of water into 20 to 30  $\mu$ m particles, by slowly dropping at room temperature while stirring with a homomixer at 7,000 r.p.m. After stirring for 20 minutes, 2 cc of an aqueous solution of 10 percent by weight of ethylene diamine were added to the dispersion while stirring at 3,000 r.p.m. in order to form microcapsules containing, as the core constituent, trichloroethylene solution of organo polysiloxane prepolymer and Catalyst. The microcapsules obtained thus were rinsed with water so as to sufficiently eliminate sodium alginate. The resultant

microcapsules had the composition and properties as shown in Table 52.

Table 52

|                                 |                  |                                                                               |
|---------------------------------|------------------|-------------------------------------------------------------------------------|
| Composition                     | Core constituent | Solution organo polysiloxane prepolymer, and Catalyst PD in trichloroethylene |
|                                 | Wall constituent | Polyurethane                                                                  |
| Ratio by weight of wall to core |                  | 1:1,000                                                                       |
| Tenacity at break               |                  | 5 g/cm <sup>2</sup>                                                           |
| Size                            |                  | 20 - 30 $\mu$ m                                                               |

A triple interlock knitted fabric made up of false twisted polycapramide textures filament yarns was impregnated with an aqueous suspension of the microcapsules and squeezed in the same manner as indicated in Example 24. Thus, the fabric was impregnated with the core constituent solution flowing out from the broken microcapsules. The fabric was dried at 100°C temperature and then heat-treated at 160°C temperature for 1 minutes. The broken wall constituents of the microcapsules could not found on the fabric by the naked eye. The resultant fabric had a superior elasticity.

## EXAMPLE 28

A solution of 0.3 part of terephthaloyl chloride and 40.0 parts of Scotchgard FC-310 in 59.5 parts of trichloroethylene was finely dispersed into an aqueous solution of 0.8 part of carboxymethyl cellulose in 400 parts of water into 10 to 30  $\mu$ m particles by slowly dropping at room temperature while stirring with a homomixer at 8,000 r.p.m. After stirring for 20 minutes, 0.5 part of hexamethylene diamine was added to the dispersion so as to form microcapsules. The obtained microcapsules were sufficiently washed with water in order to remove carboxymethyl cellulose. The resultant microcapsules had the composition and properties as shown in Table 53.

Table 53

|                                 |                  |                                                    |
|---------------------------------|------------------|----------------------------------------------------|
| Composition                     | Core Constituent | Solution of Scotchgard FC-310 in trichloroethylene |
|                                 | Wall constituent | Polyamide                                          |
| Ratio by weight of wall to core |                  | 1:1,000                                            |
| Tenacity at break               |                  | 3 g/cm <sup>2</sup>                                |
| Size                            |                  | 20 - 30 $\mu$ m                                    |

A tricot fabric made up of polyethylene terephthalate filament textured yarn was impregnated with an aqueous suspension of the microcapsules and squeezed in accordance with the manner as indicated in Example 24. The fabric was dried at 100°C temperature and then heat-treated at 150°C temperature for 3 minutes. The resultant fabric had superior water and oil repellent properties and soil proof property.

## EXAMPLE 29

A non-aqueous solvent solution was prepared by dissolving 30 parts of urethane prepolymer which was obtained through a reaction between 1 mol of polycaprolactone diol having a molecular weight of 1,500 consisting of  $\epsilon$ -caprolactone, methyl  $\epsilon$ -caprolactone

and methyl diethanol amine, 2 mol of hexamethylene diisocyanate and 1 mol of 1,3-propylene diamine into 70 parts of trichloroethylene.

The solution was dispersed into an aqueous solution containing 5 percent by weight of hydroxyethyl cellulose by slowly being dropped at room temperature while stirring at 8,000 r.p.m. into 20 to 30  $\mu$ m size particles. After completing the dispersing, 8 cc of an aqueous solution containing 10 percent by weight of ethylene diamine was added to the dispersion while stirring at 3,000 r.p.m. for 10 minutes.

The resultant microcapsules had the composition and properties as shown in FIG. 54.

Table 54

|                                 |                  |                                                      |
|---------------------------------|------------------|------------------------------------------------------|
| Composition                     | Core constituent | Solution of urethane prepolymer in trichloroethylene |
|                                 | Wall constituent | Polyurethane                                         |
| Ratio by weight of wall to core |                  | 1:1,000                                              |
| Tenacity at break               |                  | 5 g/cm <sup>2</sup>                                  |
| Size                            |                  | 20 - 30 $\mu$ m                                      |

15 The microcapsules thus prepared was washed to completely remove hydroxyethyl cellulose.

For comparison, the trichloroethylene solution as stated above, was dispersed into an aqueous solution containing 2 percent by weight of gelatin.

20 However, the trichloroethylene solution was so insufficiently dispersed as to obtain no microcapsules.

The microcapsules of the present Example were applied to a polycapramide tricot fabric from an aqueous suspension thereof through a padding process. The fabric was pressed by a pair of rubber rollers in the same manner as that of the Example 24. The impregnated fabric with the urethane prepolymer was dried at 100°C temperature and then heat-treated at 150°C temperature for 2 minutes. The resultant fabric had a superior 25 increase recovery.

What we claim is:

1. A process for treating a fibrous article selected from yarns, knitted fabrics, woven fabrics or non-woven fabrics consisting of at least one kind of natural or artificial fibers, comprising the steps of:

1. forming a suspension, in water, of a multitude of discrete microcapsules having particle sizes in the range of 100 to 1  $\mu$ m, each microcapsule consisting essentially of:

a. a liquid core consisting essentially of a solution of at least one hydrophobic fiber treating agent dissolved in a non-aqueous solvent which is not miscible with water, said fiber treating agent comprising elasticity-improving agents, anti-pilling agents, ultra-violet ray absorbers, softening agents, flame proof agents, anti-static agents, water repellent agents, soil-releasing agents, heat proof agents, shrink proof agents, crease proof agents, cross-linking agents, dyes or pigments and being capable of being adhered, absorbed or reacted with said fibers upon contact therewith, and

b. a solid, thin synthetic resin shell deposited on and completely surrounding said core, said resin being selected from the group consisting of polyurethane resins, silicone resins, polyolefins, epoxy resins, polyamides and polyesters, said

- shell having a breaking tenacity of not in excess of 50 g/cm<sup>2</sup>, the weight ratio of (b) to (a) being in the range of 1:500 to 1:5,000;
2. applying the suspension of said microcapsules in water onto said fibrous article; and
  3. breaking the microcapsules on said fibrous article to impregnate said article with said solution whereby said fibrous article is treated by said fiber treating agent.
2. A process as claimed in claim 1, wherein said non-aqueous solvent is selected from the group consisting of tetrachloromethane, tetrachloroethylene, trichloroethylene, xylene, toluene, 1,1,1-trichloroethane, benzene, ethylbenzene, industrial gasoline, chloroform, methylene chloride and tetrachloroethane and mixtures thereof.
3. A process as claimed in claim 1, wherein the maximum size of said microcapsule is not in excess of 30  $\mu$ m.
4. A process as claimed in claim 1, wherein said microcapsules contain two or more kinds of treating agents.
5. A process as claimed in claim 1, wherein said aqueous suspension of said microcapsules contains in addition at least one member selected from moistening agents, antistatic agents or dyes.
6. A process as claimed in claim 1, wherein said microcapsules are applied in an amount in the range of 5 to 400 percent based on the weight of said fibrous article.
7. A process as claimed in claim 1, wherein after said microcapsules are subjected to breaking, the treated fibrous article is subjected to heat treatment.
8. A process as claimed in claim 1, in which said fiber treating agent is a urethane prepolymer effective to improve the antipilling or the crease proof properties of the fibrous article.
9. A process as claimed in claim 1, in which the fiber treating agent is an organosiloxane prepolymer effective to improve the elasticity or the crease recovery of the fibrous article.

10. A process as claimed in claim 1, in which the fiber treating agent is dimethyl polysiloxane effective to improve the softness of the fibrous article.
11. A process as claimed in claim 1, in which the fiber treating agent is dimethyl polysiloxane diol effective to improve the softness, elasticity, water repellency, heat proofness or anti-shrinking properties of the fibrous article.
12. A process as claimed in claim 1, in which the fiber treating agent is methylhydrogen polysiloxane effective to improve the water repellency of the fibrous article.
13. A process as claimed in claim 4, wherein said microcapsules in said suspension consist of a mixture of two or more kinds of microcapsules containing different treating agents.
14. A process as claimed in claim 4, wherein all said microcapsules contain a mixture of two or more treating agents.
15. A process as claimed in claim 5, wherein said moistening agent is selected from the group consisting of addition compounds in which 2 to 50 mols of ethylene oxide is added to  $\epsilon$ -caprolactam, addition compounds in which 2 to 50 mols of propylene oxide is added to  $\epsilon$ -caprolactam, addition compounds in which 2 to 50 mols of propylene oxide is added to oligomer of  $\epsilon$ -caprolactam, sodium N-acyl aminoacetate, sodium N-acyl- $\alpha$ -aminopropionate and sodium N-acyl- $\beta$ -aminopropionate.
16. A process as claimed in claim 6, wherein said microcapsules are applied in an amount in the range of from 10 to 100 percent based on the weight of said fibrous articles.
17. A process as claimed in claim 7, wherein said heat treatment is carried out at a room temperature of 50° to 200°C.
18. A process as claimed in claim 17, wherein said temperature of said heat treatment is in a range of from 80° to 180°C.

\* \* \* \* \*

UNITED STATES PATENT OFFICE  
CERTIFICATE OF CORRECTION

Patent No. 3 870 542 Dated March 11, 1975

Inventor(s) Syunya Ida and Kenjiro Hosokawa

It is certified that error appears in the above-identified patent and that said Letters Patent are hereby corrected as shown below:

Col. 38, line 35; please change "room temperature" to read  
---temperature---.

Signed and sealed this 17th day of June 1975.

(SEAL)

Attest:

RUTH C. MASON  
Attesting Officer

C. MARSHALL DANN  
Commissioner of Patents  
and Trademarks